



US010221637B2

(12) **United States Patent**  
**Xu et al.**

(10) **Patent No.:** **US 10,221,637 B2**  
(45) **Date of Patent:** **\*Mar. 5, 2019**

(54) **METHODS OF MANUFACTURING DISSOLVABLE TOOLS VIA LIQUID-SOLID STATE MOLDING**

(71) Applicants: **Zhiyue Xu**, Cypress, TX (US); **Bobby Salinas**, Sugar Land, TX (US); **Zhihui Zhang**, Katy, TX (US)

(72) Inventors: **Zhiyue Xu**, Cypress, TX (US); **Bobby Salinas**, Sugar Land, TX (US); **Zhihui Zhang**, Katy, TX (US)

(73) Assignee: **BAKER HUGHES, A GE COMPANY, LLC**, Houston, TX (US)

(\*) Notice: Subject to any disclaimer, the term of this patent is extended or adjusted under 35 U.S.C. 154(b) by 204 days.

This patent is subject to a terminal disclaimer.

(21) Appl. No.: **14/823,491**

(22) Filed: **Aug. 11, 2015**

(65) **Prior Publication Data**

US 2017/0044675 A1 Feb. 16, 2017

(51) **Int. Cl.**

**E21B 23/00** (2006.01)  
**B22D 1/00** (2006.01)  
**B22D 17/00** (2006.01)  
**B22D 19/06** (2006.01)  
**B22D 19/14** (2006.01)  
**B22D 21/00** (2006.01)  
**B22D 27/02** (2006.01)  
**B22D 27/08** (2006.01)

(52) **U.S. Cl.**

CPC ..... **E21B 23/00** (2013.01); **B22D 1/007** (2013.01); **B22D 17/007** (2013.01); **B22D 19/06** (2013.01); **B22D 19/14** (2013.01); **B22D 21/00** (2013.01); **B22D 27/02** (2013.01); **B22D 27/08** (2013.01)

(58) **Field of Classification Search**

CPC ..... E21B 23/00; B22D 1/007; B22D 17/007; B22D 19/06; B22D 19/14; B22D 21/00; B22D 27/02; B22D 27/08

See application file for complete search history.

(56) **References Cited**

U.S. PATENT DOCUMENTS

|             |         |               |
|-------------|---------|---------------|
| 1,468,905 A | 9/1923  | Herman        |
| 1,558,066 A | 10/1925 | Veazey et al. |
| 2,189,697 A | 2/1940  | Baker         |
| 2,222,233 A | 11/1940 | Mize          |
| 2,225,143 A | 12/1940 | Baker et al.  |
| 2,238,895 A | 4/1941  | Gage          |
| 2,261,292 A | 11/1941 | Salnikov      |
| 2,294,648 A | 9/1942  | Ansel         |
| 2,301,624 A | 11/1942 | Holt          |
| 2,352,993 A | 7/1944  | Albertson     |
| 2,394,843 A | 2/1946  | Cooke et al.  |
| 2,672,199 A | 3/1954  | McKenna       |

|             |         |                   |
|-------------|---------|-------------------|
| 2,753,941 A | 7/1956  | Hebard et al.     |
| 2,754,910 A | 7/1956  | Derrick et al.    |
| 2,933,136 A | 4/1960  | Ayers et al.      |
| 2,983,634 A | 5/1961  | Budininkas et al. |
| 3,057,405 A | 10/1962 | Mallinger         |
| 3,066,391 A | 12/1962 | Vordahl           |
| 3,106,959 A | 10/1963 | Huitt et al.      |
| 3,142,338 A | 7/1964  | Brown             |
| 3,152,009 A | 10/1964 | Delong            |
| 3,180,728 A | 4/1965  | Keir et al.       |
| 3,196,949 A | 7/1965  | Thomas            |
| 3,226,314 A | 12/1965 | Wellington et al. |
| 3,242,988 A | 3/1966  | McGuire et al.    |
| 3,316,748 A | 5/1967  | Lang et al.       |
| 3,326,291 A | 6/1967  | Zandmer et al.    |
| 3,343,537 A | 9/1967  | Graham            |
| 3,347,317 A | 10/1967 | Zandemer          |
| 3,347,714 A | 10/1967 | Broverman et al.  |
| 3,390,724 A | 7/1968  | Caldwell          |
| 3,395,758 A | 8/1968  | Kelly et al.      |
| 3,406,101 A | 10/1968 | Kilpatrick        |
| 3,416,918 A | 12/1968 | Roberts           |
| 3,465,181 A | 9/1969  | Colby et al.      |
| 3,489,218 A | 1/1970  | Means             |
| 3,513,230 A | 5/1970  | Rhees et al.      |
| 3,600,163 A | 8/1971  | Badia et al.      |
| 3,602,305 A | 8/1971  | Kisling           |
| 3,637,446 A | 1/1972  | Elliott et al.    |
| 3,645,331 A | 2/1972  | Maurer et al.     |
| 3,660,049 A | 5/1972  | Benjamin          |
| 3,765,484 A | 10/1973 | Hamby, Jr. et al. |
| 3,768,563 A | 10/1973 | Blount            |
| 3,775,823 A | 12/1973 | Adolph et al.     |
| 3,816,080 A | 6/1974  | Bomford et al.    |
| 3,878,889 A | 4/1975  | Seabourn          |
| 3,894,850 A | 7/1975  | Kovalchuk et al.  |
| 3,924,677 A | 12/1975 | Prenner et al.    |
| 3,957,483 A | 5/1976  | Suzuki            |
| 4,010,583 A | 3/1977  | Highborg          |
| 4,039,717 A | 8/1977  | Titus             |
| 4,050,529 A | 9/1977  | Tagirov et al.    |
| 4,157,732 A | 6/1979  | Fonner            |

(Continued)

FOREIGN PATENT DOCUMENTS

|    |            |        |
|----|------------|--------|
| CA | 2783241 A1 | 6/2011 |
| CA | 2783346 A1 | 6/2011 |

(Continued)

OTHER PUBLICATIONS

"Declaration of Karl T. Hartwig in Support of Petitioner Pursuant to 37 C.F.R. § 42.120", executed on Nov. 21, 2016 in support of U.S. Pat. No. 8,573,295, 52 pages.

(Continued)

Primary Examiner — Patrick D Niland

(74) Attorney, Agent, or Firm — Cantor Colburn LLP

(57)

**ABSTRACT**

A method of manufacturing a dissolvable article comprises forming a liquid-solid mixture comprising secondary particles homogeneously dispersed in a molten metallic matrix material; disposing the liquid-solid mixture in a mold; agitating the liquid-solid mixture in the mold; and molding the liquid-solid mixture under agitation to form a dissolvable article, wherein the secondary particles and the metallic matrix material form a plurality of micro- or nano-sized galvanic cells in the dissolvable article.

21 Claims, 2 Drawing Sheets

| (56)                  | References Cited |                       |             |         |                          |
|-----------------------|------------------|-----------------------|-------------|---------|--------------------------|
| U.S. PATENT DOCUMENTS |                  |                       |             |         |                          |
| 4,248,307 A           | 2/1981           | Silberman et al.      | 5,010,955 A | 4/1991  | Springer                 |
| 4,284,137 A           | 8/1981           | Taylor                | 5,036,921 A | 8/1991  | Pittard et al.           |
| 4,292,377 A           | 9/1981           | Petersen et al.       | 5,048,611 A | 9/1991  | Cochran                  |
| 4,372,384 A           | 2/1983           | Kinney                | 5,049,165 A | 9/1991  | Tselesin                 |
| 4,373,584 A           | 2/1983           | Silberman et al.      | 5,061,323 A | 10/1991 | Deluccia                 |
| 4,373,952 A           | 2/1983           | Parent                | 5,063,775 A | 11/1991 | Walker, Sr. et al.       |
| 4,374,543 A           | 2/1983           | Richardson            | 5,073,207 A | 12/1991 | Faure et al.             |
| 4,384,616 A           | 5/1983           | Dellinger             | 5,074,361 A | 12/1991 | Brisco et al.            |
| 4,395,440 A           | 7/1983           | Abe et al.            | 5,076,869 A | 12/1991 | Bourell et al.           |
| 4,399,871 A           | 8/1983           | Adkins et al.         | 5,084,088 A | 1/1992  | Okazaki                  |
| 4,407,368 A           | 10/1983          | Erbstoesser           | 5,087,304 A | 2/1992  | Chang et al.             |
| 4,422,508 A           | 12/1983          | Rutledge, Jr. et al.  | 5,090,480 A | 2/1992  | Pittard et al.           |
| 4,450,136 A           | 5/1984           | Dudek et al.          | 5,095,988 A | 3/1992  | Bode                     |
| 4,452,311 A           | 6/1984           | Speegle et al.        | 5,103,911 A | 4/1992  | Heijnen                  |
| 4,475,729 A           | 10/1984          | Costigan              | 5,117,915 A | 6/1992  | Mueller et al.           |
| 4,498,543 A           | 2/1985           | Pye et al.            | 5,161,614 A | 11/1992 | Wu et al.                |
| 4,499,048 A           | 2/1985           | Hanejko               | 5,171,734 A | 12/1992 | Sanjurjo et al.          |
| 4,499,049 A           | 2/1985           | Hanejko               | 5,178,216 A | 1/1993  | Giroux et al.            |
| 4,524,825 A           | 6/1985           | Fore                  | 5,181,571 A | 1/1993  | Mueller et al.           |
| 4,526,840 A           | 7/1985           | Jerabek               | 5,183,631 A | 2/1993  | Kugimiya et al.          |
| 4,534,414 A           | 8/1985           | Pringle               | 5,188,182 A | 2/1993  | Echols, III et al.       |
| 4,539,175 A           | 9/1985           | Lichti et al.         | 5,188,183 A | 2/1993  | Hopmann et al.           |
| 4,554,986 A           | 11/1985          | Jones                 | 5,204,055 A | 4/1993  | Sachs et al.             |
| 4,619,699 A           | 10/1986          | Petkovic-Luton et al. | 5,222,867 A | 6/1993  | Walker, Sr. et al.       |
| 4,640,354 A           | 2/1987           | Boisson               | 5,226,483 A | 7/1993  | Williamson, Jr.          |
| 4,648,901 A           | 3/1987           | Murray et al.         | 5,228,518 A | 7/1993  | Wilson et al.            |
| 4,664,962 A           | 5/1987           | Desmarais, Jr.        | 5,234,055 A | 8/1993  | Cornette                 |
| 4,668,470 A           | 5/1987           | Gilman et al.         | 5,240,742 A | 8/1993  | Johnson ..... B22F 1/025 |
| 4,673,549 A           | 6/1987           | Ecer                  |             |         | 427/216                  |
| 4,674,572 A           | 6/1987           | Gallus                | 5,252,365 A | 10/1993 | White                    |
| 4,678,037 A           | 7/1987           | Smith                 | 5,253,714 A | 10/1993 | Davis et al.             |
| 4,681,133 A           | 7/1987           | Weston                | 5,271,468 A | 12/1993 | Streich et al.           |
| 4,688,641 A           | 8/1987           | Knieriem              | 5,273,569 A | 12/1993 | Gilman et al.            |
| 4,690,796 A           | 9/1987           | Paliwal               | 5,282,509 A | 2/1994  | Schurr, III              |
| 4,693,863 A           | 9/1987           | Del Corso et al.      | 5,292,478 A | 3/1994  | Scorey                   |
| 4,703,807 A           | 11/1987          | Weston                | 5,293,940 A | 3/1994  | Hromas et al.            |
| 4,706,753 A           | 11/1987          | Ohkochi et al.        | 5,304,260 A | 4/1994  | Aikawa et al.            |
| 4,708,202 A           | 11/1987          | Sukup et al.          | 5,304,588 A | 4/1994  | Boysen et al.            |
| 4,708,208 A           | 11/1987          | Halbardier            | 5,309,874 A | 5/1994  | Willermet et al.         |
| 4,709,761 A           | 12/1987          | Setterberg, Jr.       | 5,310,000 A | 5/1994  | Arterbury et al.         |
| 4,714,116 A           | 12/1987          | Brunner               | 5,316,598 A | 5/1994  | Chang et al.             |
| 4,716,964 A           | 1/1988           | Erbstoesser et al.    | 5,318,746 A | 6/1994  | Lashmore                 |
| 4,719,971 A           | 1/1988           | Owens                 | 5,352,522 A | 10/1994 | Kugimiya et al.          |
| 4,721,159 A           | 1/1988           | Ohkochi et al.        | 5,380,473 A | 1/1995  | Bogue et al.             |
| 4,738,599 A           | 4/1988           | Shilling              | 5,387,380 A | 2/1995  | Cima et al.              |
| 4,741,973 A           | 5/1988           | Condit et al.         | 5,392,860 A | 2/1995  | Ross                     |
| 4,768,588 A           | 9/1988           | Kupsa                 | 5,394,236 A | 2/1995  | Murnick                  |
| 4,775,598 A           | 10/1988          | Jaekel                | 5,394,941 A | 3/1995  | Venditto et al.          |
| 4,784,226 A           | 11/1988          | Wyatt                 | 5,398,754 A | 3/1995  | Dinhoble                 |
| 4,805,699 A           | 2/1989           | Halbardier            | 5,407,011 A | 4/1995  | Layout                   |
| 4,817,725 A           | 4/1989           | Jenkins               | 5,409,555 A | 4/1995  | Fujita et al.            |
| 4,834,184 A           | 5/1989           | Streich et al.        | 5,411,082 A | 5/1995  | Kennedy                  |
| H635 H                | 6/1989           | Johnson et al.        | 5,417,285 A | 5/1995  | Van Buskirk et al.       |
| 4,850,432 A           | 7/1989           | Porter et al.         | 5,425,424 A | 6/1995  | Reinhardt et al.         |
| 4,853,056 A           | 8/1989           | Hoffman               | 5,427,177 A | 6/1995  | Jordan, Jr. et al.       |
| 4,869,324 A           | 9/1989           | Holder                | 5,435,392 A | 7/1995  | Kennedy                  |
| 4,869,325 A           | 9/1989           | Halbardier            | 5,439,051 A | 8/1995  | Kennedy et al.           |
| 4,880,059 A           | 11/1989          | Brandell et al.       | 5,445,430 A | 10/1995 | Kennedy et al.           |
| 4,889,187 A           | 12/1989          | Terrell et al.        | 5,456,317 A | 10/1995 | Hood, III et al.         |
| 4,890,675 A           | 1/1990           | Dew                   | 5,456,327 A | 10/1995 | Denton et al.            |
| 4,901,794 A           | 2/1990           | Baugh et al.          | 5,464,062 A | 11/1995 | Blizzard, Jr.            |
| 4,909,320 A           | 3/1990           | Hebert et al.         | 5,472,048 A | 12/1995 | Kennedy et al.           |
| 4,921,664 A           | 5/1990           | Couper                | 5,474,131 A | 12/1995 | Jordan, Jr. et al.       |
| 4,929,415 A           | 5/1990           | Okazaki               | 5,477,923 A | 12/1995 | Jordan, Jr. et al.       |
| 4,932,474 A           | 6/1990           | Schroeder, Jr. et al. | 5,479,986 A | 1/1996  | Gano et al.              |
| 4,938,309 A           | 7/1990           | Emdy                  | 5,506,055 A | 4/1996  | Dorfman et al.           |
| 4,944,351 A           | 7/1990           | Eriksen et al.        | 5,507,439 A | 4/1996  | Story                    |
| 4,949,788 A           | 8/1990           | Szarka et al.         | 5,511,620 A | 4/1996  | Baugh et al.             |
| 4,952,902 A           | 8/1990           | Kawaguchi et al.      | 5,524,699 A | 6/1996  | Cook                     |
| 4,975,412 A           | 12/1990          | Okazaki et al.        | 5,526,880 A | 6/1996  | Jordan, Jr. et al.       |
| 4,977,958 A           | 12/1990          | Miller                | 5,526,881 A | 6/1996  | Martin et al.            |
| 4,981,177 A           | 1/1991           | Carmody et al.        | 5,529,746 A | 6/1996  | Knoss et al.             |
| 4,986,361 A           | 1/1991           | Mueller et al.        | 5,533,573 A | 7/1996  | Jordan, Jr. et al.       |
| 4,997,622 A           | 3/1991           | Regazzoni et al.      | 5,536,485 A | 7/1996  | Kume et al.              |
| 5,006,044 A           | 4/1991           | Walker, Sr. et al.    | 5,558,153 A | 9/1996  | Holcombe et al.          |
|                       |                  |                       | 5,601,924 A | 2/1997  | Beane                    |
|                       |                  |                       | 5,607,017 A | 3/1997  | Owens et al.             |
|                       |                  |                       | 5,623,993 A | 4/1997  | Van Buskirk et al.       |
|                       |                  |                       | 5,623,994 A | 4/1997  | Robinson                 |

| (56)                  | References Cited |                    |              |         |                     |  |
|-----------------------|------------------|--------------------|--------------|---------|---------------------|--|
| U.S. PATENT DOCUMENTS |                  |                    |              |         |                     |  |
| 5,636,691 A           | 6/1997           | Hendrickson et al. | 6,341,747 B1 | 1/2002  | Schmidt et al.      |  |
| 5,641,023 A           | 6/1997           | Ross et al.        | 6,349,766 B1 | 2/2002  | Bussear et al.      |  |
| 5,647,444 A           | 7/1997           | Williams           | 6,354,372 B1 | 3/2002  | Carisella et al.    |  |
| 5,665,289 A           | 9/1997           | Chung et al.       | 6,354,379 B2 | 3/2002  | Miszewski et al.    |  |
| 5,677,372 A           | 10/1997          | Yamamoto et al.    | 6,357,322 B1 | 3/2002  | Dolan et al.        |  |
| 5,685,372 A           | 11/1997          | Gano               | 6,357,332 B1 | 3/2002  | Vecchio             |  |
| 5,701,576 A           | 12/1997          | Fujita et al.      | 6,371,206 B1 | 4/2002  | Mills               |  |
| 5,707,214 A           | 1/1998           | Schmidt            | 6,372,346 B1 | 4/2002  | Toth                |  |
| 5,709,269 A           | 1/1998           | Head               | 6,382,244 B2 | 5/2002  | Vann                |  |
| 5,720,344 A           | 2/1998           | Newman             | 6,390,195 B1 | 5/2002  | Nguyen et al.       |  |
| 5,722,033 A           | 2/1998           | Carden             | 6,390,200 B1 | 5/2002  | Allamon et al.      |  |
| 5,728,195 A           | 3/1998           | Eastman et al.     | 6,394,180 B1 | 5/2002  | Berscheidt et al.   |  |
| 5,765,639 A           | 6/1998           | Muth               | 6,394,185 B1 | 5/2002  | Constien            |  |
| 5,772,735 A           | 6/1998           | Sehgal et al.      | 6,397,950 B1 | 6/2002  | Streich et al.      |  |
| 5,782,305 A           | 7/1998           | Hicks              | 6,401,547 B1 | 6/2002  | Hatfield et al.     |  |
| 5,797,454 A           | 8/1998           | Hipp               | 6,403,210 B1 | 6/2002  | Stuivinga et al.    |  |
| 5,826,652 A           | 10/1998          | Tapp               | 6,408,946 B1 | 6/2002  | Marshall et al.     |  |
| 5,826,661 A           | 10/1998          | Parker et al.      | 6,419,023 B1 | 7/2002  | George et al.       |  |
| 5,829,520 A           | 11/1998          | Johnson            | 6,439,313 B1 | 8/2002  | Thomeer et al.      |  |
| 5,836,396 A           | 11/1998          | Norman             | 6,446,717 B1 | 9/2002  | White et al.        |  |
| 5,857,521 A           | 1/1999           | Ross et al.        | 6,457,525 B1 | 10/2002 | Scott               |  |
| 5,881,816 A           | 3/1999           | Wright             | 6,467,546 B2 | 10/2002 | Allamon et al.      |  |
| 5,896,819 A           | 4/1999           | Turila et al.      | 6,470,965 B1 | 10/2002 | Winzer              |  |
| 5,902,424 A           | 5/1999           | Fujita et al.      | 6,491,097 B1 | 12/2002 | Oneal et al.        |  |
| 5,934,372 A           | 8/1999           | Muth               | 6,491,116 B2 | 12/2002 | Berscheidt et al.   |  |
| 5,941,309 A           | 8/1999           | Appleton           | 6,513,598 B2 | 2/2003  | Moore et al.        |  |
| 5,960,881 A           | 10/1999          | Allamon et al.     | 6,513,600 B2 | 2/2003  | Ross                |  |
| 5,964,965 A           | 10/1999          | Schulz et al.      | 6,540,033 B1 | 4/2003  | Sullivan et al.     |  |
| 5,985,466 A           | 11/1999          | Atarashi et al.    | 6,543,543 B2 | 4/2003  | Muth                |  |
| 5,988,287 A           | 11/1999          | Jordan, Jr. et al. | 6,561,275 B2 | 5/2003  | Glass et al.        |  |
| 5,990,051 A           | 11/1999          | Ischy et al.       | 6,588,507 B2 | 7/2003  | Dusterhoft et al.   |  |
| 5,992,452 A           | 11/1999          | Nelson, II         | 6,591,915 B2 | 7/2003  | Burris et al.       |  |
| 5,992,520 A           | 11/1999          | Schultz et al.     | 6,601,648 B2 | 8/2003  | Ebinger             |  |
| 6,007,314 A           | 12/1999          | Nelson, II         | 6,601,650 B2 | 8/2003  | Sundararajan        |  |
| 6,024,915 A           | 2/2000           | Kume et al.        | 6,609,569 B2 | 8/2003  | Howlett et al.      |  |
| 6,032,735 A           | 3/2000           | Echols             | 6,612,826 B1 | 9/2003  | Bauer et al.        |  |
| 6,036,777 A           | 3/2000           | Sachs              | 6,613,383 B1 | 9/2003  | George et al.       |  |
| 6,047,773 A           | 4/2000           | Zeltmann et al.    | 6,619,400 B2 | 9/2003  | Brunet              |  |
| 6,050,340 A           | 4/2000           | Scott              | 6,634,428 B2 | 10/2003 | Krauss et al.       |  |
| 6,069,313 A           | 5/2000           | Kay                | 6,662,886 B2 | 12/2003 | Russell             |  |
| 6,076,600 A           | 6/2000           | Vick, Jr. et al.   | 6,675,889 B1 | 1/2004  | Mullins et al.      |  |
| 6,079,496 A           | 6/2000           | Hirth              | 6,699,305 B2 | 3/2004  | Myrick              |  |
| 6,085,837 A           | 7/2000           | Massinon et al.    | 6,712,153 B2 | 3/2004  | Turley et al.       |  |
| 6,095,247 A           | 8/2000           | Streich et al.     | 6,712,797 B1 | 3/2004  | Southern, Jr.       |  |
| 6,119,783 A           | 9/2000           | Parker et al.      | 6,713,177 B2 | 3/2004  | George et al.       |  |
| 6,142,237 A           | 11/2000          | Christmas et al.   | 6,715,541 B2 | 4/2004  | Pedersen et al.     |  |
| 6,161,622 A           | 12/2000          | Robb               | 6,719,051 B2 | 4/2004  | Hailey, Jr. et al.  |  |
| 6,167,970 B1          | 1/2001           | Stout et al.       | 6,755,249 B2 | 6/2004  | Robison et al.      |  |
| 6,170,583 B1          | 1/2001           | Boyce              | 6,769,491 B2 | 8/2004  | Zimmerman et al.    |  |
| 6,173,779 B1          | 1/2001           | Smith              | 6,776,228 B2 | 8/2004  | Pedersen et al.     |  |
| 6,176,323 B1          | 1/2001           | Weirich et al.     | 6,779,599 B2 | 8/2004  | Mullins et al.      |  |
| 6,189,616 B1          | 2/2001           | Gano et al.        | 6,799,638 B2 | 10/2004 | Butterfield, Jr.    |  |
| 6,189,618 B1          | 2/2001           | Beeman et al.      | 6,810,960 B2 | 11/2004 | Pia                 |  |
| 6,213,202 B1          | 4/2001           | Read, Jr.          | 6,817,414 B2 | 11/2004 | Lee                 |  |
| 6,220,350 B1          | 4/2001           | Brothers et al.    | 6,831,044 B2 | 12/2004 | Constien            |  |
| 6,220,357 B1          | 4/2001           | Carmichael et al.  | 6,883,611 B2 | 4/2005  | Smith et al.        |  |
| 6,228,904 B1          | 5/2001           | Yadav et al.       | 6,887,297 B2 | 5/2005  | Winter et al.       |  |
| 6,237,688 B1          | 5/2001           | Burleson et al.    | 6,896,049 B2 | 5/2005  | Moyes               |  |
| 6,238,280 B1          | 5/2001           | Ritt et al.        | 6,896,061 B2 | 5/2005  | Hriscu et al.       |  |
| 6,241,021 B1          | 6/2001           | Bowling            | 6,899,176 B2 | 5/2005  | Hailey, Jr. et al.  |  |
| 6,248,399 B1          | 6/2001           | Hehmann            | 6,899,777 B2 | 5/2005  | Vaidyanathan et al. |  |
| 6,250,392 B1          | 6/2001           | Muth               | 6,908,516 B2 | 6/2005  | Hehmann et al.      |  |
| 6,261,432 B1          | 7/2001           | Huber et al.       | 6,913,827 B2 | 7/2005  | George et al.       |  |
| 6,265,205 B1          | 7/2001           | Hitchens et al.    | 6,926,086 B2 | 8/2005  | Patterson et al.    |  |
| 6,273,187 B1          | 8/2001           | Voisin, Jr. et al. | 6,932,159 B2 | 8/2005  | Hovem               |  |
| 6,276,452 B1          | 8/2001           | Davis et al.       | 6,939,388 B2 | 9/2005  | Angeliu             |  |
| 6,276,457 B1          | 8/2001           | Moffatt et al.     | 6,945,331 B2 | 9/2005  | Patel               |  |
| 6,279,656 B1          | 8/2001           | Sinclair et al.    | 6,951,331 B2 | 10/2005 | Haughom et al.      |  |
| 6,287,445 B1          | 9/2001           | Lashmore et al.    | 6,959,759 B2 | 11/2005 | Doane et al.        |  |
| 6,302,205 B1          | 10/2001          | Ryll               | 6,973,970 B2 | 12/2005 | Johnston et al.     |  |
| 6,315,041 B1          | 11/2001          | Carlisle et al.    | 6,973,973 B2 | 12/2005 | Howard et al.       |  |
| 6,315,050 B2          | 11/2001          | Vaynshteyn et al.  | 6,983,796 B2 | 1/2006  | Bayne et al.        |  |
| 6,325,148 B1          | 12/2001          | Trahan et al.      | 6,986,390 B2 | 1/2006  | Doane et al.        |  |
| 6,328,110 B1          | 12/2001          | Joubert            | 7,013,989 B2 | 3/2006  | Hammond et al.      |  |
| 6,341,653 B1          | 1/2002           | Firmaniuk et al.   | 7,013,998 B2 | 3/2006  | Ray et al.          |  |
|                       |                  |                    | 7,017,664 B2 | 3/2006  | Walker et al.       |  |
|                       |                  |                    | 7,017,677 B2 | 3/2006  | Keshavan et al.     |  |
|                       |                  |                    | 7,021,389 B2 | 4/2006  | Bishop et al.       |  |
|                       |                  |                    | 7,025,146 B2 | 4/2006  | King et al.         |  |

| (56)                  | References Cited              |              |                             |  |  |
|-----------------------|-------------------------------|--------------|-----------------------------|--|--|
| U.S. PATENT DOCUMENTS |                               |              |                             |  |  |
| 7,028,778 B2          | 4/2006 Krywitsky              | 7,552,779 B2 | 6/2009 Murray               |  |  |
| 7,044,230 B2          | 5/2006 Starr et al.           | 7,559,357 B2 | 7/2009 Clem                 |  |  |
| 7,049,272 B2          | 5/2006 Sinclair et al.        | 7,575,062 B2 | 8/2009 East, Jr.            |  |  |
| 7,051,805 B2          | 5/2006 Doane et al.           | 7,579,087 B2 | 8/2009 Maloney et al.       |  |  |
| 7,059,410 B2          | 6/2006 Bousche et al.         | 7,591,318 B2 | 9/2009 Tilghman             |  |  |
| 7,090,027 B1          | 8/2006 Williams               | 7,600,572 B2 | 10/2009 Slup et al.         |  |  |
| 7,093,664 B2          | 8/2006 Todd et al.            | 7,604,049 B2 | 10/2009 Vaidya et al.       |  |  |
| 7,096,945 B2          | 8/2006 Richards et al.        | 7,604,055 B2 | 10/2009 Richard et al.      |  |  |
| 7,096,946 B2          | 8/2006 Jasser et al.          | 7,607,476 B2 | 10/2009 Tom et al.          |  |  |
| 7,097,807 B1          | 8/2006 Meeks, III et al.      | 7,617,871 B2 | 11/2009 Surjaatmadja et al. |  |  |
| 7,097,906 B2          | 8/2006 Gardner                | 7,635,023 B2 | 12/2009 Goldberg et al.     |  |  |
| 7,108,080 B2          | 9/2006 Tessari et al.         | 7,640,988 B2 | 1/2010 Phi et al.           |  |  |
| 7,111,682 B2          | 9/2006 Blaisdell              | 7,661,480 B2 | 2/2010 Al-Anazi             |  |  |
| 7,128,145 B2          | 10/2006 Mickey                | 7,661,481 B2 | 2/2010 Todd et al.          |  |  |
| 7,141,207 B2          | 11/2006 Jandeska, Jr. et al.  | 7,665,537 B2 | 2/2010 Patel et al.         |  |  |
| 7,150,326 B2          | 12/2006 Bishop et al.         | 7,686,082 B2 | 3/2010 Marsh                |  |  |
| 7,163,066 B2          | 1/2007 Lehr                   | 7,690,436 B2 | 4/2010 Turley et al.        |  |  |
| 7,165,622 B2          | 1/2007 Hirth et al.           | 7,699,101 B2 | 4/2010 Fripp et al.         |  |  |
| 7,168,494 B2          | 1/2007 Starr et al.           | 7,703,510 B2 | 4/2010 Xu                   |  |  |
| 7,174,963 B2          | 2/2007 Bertelsen              | 7,703,511 B2 | 4/2010 Buyers et al.        |  |  |
| 7,182,135 B2          | 2/2007 Szarka                 | 7,708,078 B2 | 5/2010 Stoesz               |  |  |
| 7,188,559 B1          | 3/2007 Vecchio                | 7,709,421 B2 | 5/2010 Jones et al.         |  |  |
| 7,210,527 B2          | 5/2007 Walker et al.          | 7,712,541 B2 | 5/2010 Loretz et al.        |  |  |
| 7,210,533 B2          | 5/2007 Starr et al.           | 7,723,272 B2 | 5/2010 Crews et al.         |  |  |
| 7,217,311 B2          | 5/2007 Hong et al.            | 7,726,406 B2 | 6/2010 Xu                   |  |  |
| 7,234,530 B2          | 6/2007 Gass                   | 7,735,578 B2 | 6/2010 Loehr et al.         |  |  |
| 7,250,188 B2          | 7/2007 Dodelet et al.         | 7,743,836 B2 | 6/2010 Cook et al.          |  |  |
| 7,252,162 B2          | 8/2007 Akinlade et al.        | 7,752,971 B2 | 7/2010 Loehr                |  |  |
| 7,255,172 B2          | 8/2007 Johnson                | 7,757,773 B2 | 7/2010 Rytlewski            |  |  |
| 7,255,178 B2          | 8/2007 Slup et al.            | 7,762,342 B2 | 7/2010 Richard et al.       |  |  |
| 7,264,060 B2          | 9/2007 Wills                  | 7,770,652 B2 | 8/2010 Barnett              |  |  |
| 7,267,172 B2          | 9/2007 Hofman                 | 7,771,289 B2 | 8/2010 Palumbo et al.       |  |  |
| 7,267,178 B2          | 9/2007 Krywitsky              | 7,775,284 B2 | 8/2010 Richards et al.      |  |  |
| 7,270,186 B2          | 9/2007 Johnson                | 7,775,285 B2 | 8/2010 Surjaatmadja et al.  |  |  |
| 7,287,592 B2          | 10/2007 Surjaatmadja et al.   | 7,775,286 B2 | 8/2010 Duphorne             |  |  |
| 7,311,152 B2          | 12/2007 Howard et al.         | 7,798,226 B2 | 9/2010 Themig               |  |  |
| 7,316,274 B2          | 1/2008 Xu et al.              | 7,798,236 B2 | 9/2010 McKeachnie et al.    |  |  |
| 7,320,365 B2          | 1/2008 Pia                    | 7,806,189 B2 | 10/2010 Frazier             |  |  |
| 7,322,412 B2          | 1/2008 Badalamenti et al.     | 7,806,192 B2 | 10/2010 Foster et al.       |  |  |
| 7,322,417 B2          | 1/2008 Rytlewski et al.       | 7,810,553 B2 | 10/2010 Cruickshank et al.  |  |  |
| 7,325,617 B2          | 2/2008 Murray                 | 7,810,567 B2 | 10/2010 Daniels et al.      |  |  |
| 7,328,750 B2          | 2/2008 Swor et al.            | 7,819,198 B2 | 10/2010 Birckhead et al.    |  |  |
| 7,331,388 B2          | 2/2008 Vilela et al.          | 7,828,055 B2 | 11/2010 Willauer et al.     |  |  |
| 7,337,854 B2          | 3/2008 Horn et al.            | 7,833,944 B2 | 11/2010 Munoz et al.        |  |  |
| 7,346,456 B2          | 3/2008 Le Bemadjiel           | 7,849,927 B2 | 12/2010 Herrera             |  |  |
| 7,350,582 B2          | 4/2008 McKeachnie et al.      | 7,851,016 B2 | 12/2010 Arbab et al.        |  |  |
| 7,353,879 B2          | 4/2008 Todd et al.            | 7,855,168 B2 | 12/2010 Fuller et al.       |  |  |
| 7,360,593 B2          | 4/2008 Consten                | 7,861,779 B2 | 1/2011 Vestavik             |  |  |
| 7,360,597 B2          | 4/2008 Blaisdell              | 7,861,781 B2 | 1/2011 D'Arcy               |  |  |
| 7,363,970 B2          | 4/2008 Corre et al.           | 7,874,365 B2 | 1/2011 East, Jr. et al.     |  |  |
| 7,373,978 B2          | 5/2008 Barry et al.           | 7,878,253 B2 | 2/2011 Stowe et al.         |  |  |
| 7,384,443 B2          | 6/2008 Mirchandani            | 7,879,367 B2 | 2/2011 Heublein et al.      |  |  |
| 7,387,158 B2          | 6/2008 Murray et al.          | 7,896,091 B2 | 3/2011 Williamson et al.    |  |  |
| 7,387,165 B2          | 6/2008 Lopez De Cerdas et al. | 7,897,063 B1 | 3/2011 Perry et al.         |  |  |
| 7,392,841 B2          | 7/2008 Murray et al.          | 7,900,696 B1 | 3/2011 Nish et al.          |  |  |
| 7,401,648 B2          | 7/2008 Bennett                | 7,900,703 B2 | 3/2011 Clark et al.         |  |  |
| 7,416,029 B2          | 8/2008 Telfer et al.          | 7,909,096 B2 | 3/2011 Clark et al.         |  |  |
| 7,422,058 B2          | 9/2008 O'Malley               | 7,909,104 B2 | 3/2011 Bjorgum              |  |  |
| 7,426,964 B2          | 9/2008 Lynde et al.           | 7,909,110 B2 | 3/2011 Sharma et al.        |  |  |
| 7,441,596 B2          | 10/2008 Wood et al.           | 7,909,115 B2 | 3/2011 Grove et al.         |  |  |
| 7,445,049 B2          | 11/2008 Howard et al.         | 7,913,765 B2 | 3/2011 Crow et al.          |  |  |
| 7,451,815 B2          | 11/2008 Hailey, Jr.           | 7,918,275 B2 | 4/2011 Clem                 |  |  |
| 7,451,817 B2          | 11/2008 Reddy et al.          | 7,931,093 B2 | 4/2011 Foster et al.        |  |  |
| 7,461,699 B2          | 12/2008 Richard et al.        | 7,938,191 B2 | 5/2011 Vaidya               |  |  |
| 7,464,764 B2          | 12/2008 Xu                    | 7,946,335 B2 | 5/2011 Bewlay et al.        |  |  |
| 7,472,750 B2          | 1/2009 Walker et al.          | 7,946,340 B2 | 5/2011 Surjaatmadja et al.  |  |  |
| 7,478,676 B2          | 1/2009 East, Jr. et al.       | 7,958,940 B2 | 6/2011 Jameson              |  |  |
| 7,503,390 B2          | 3/2009 Gomez                  | 7,963,331 B2 | 6/2011 Surjaatmadja et al.  |  |  |
| 7,503,399 B2          | 3/2009 Badalamenti et al.     | 7,963,340 B2 | 6/2011 Gramstad et al.      |  |  |
| 7,509,993 B1          | 3/2009 Turng et al.           | 7,963,342 B2 | 6/2011 George               |  |  |
| 7,510,018 B2          | 3/2009 Williamson et al.      | 7,980,300 B2 | 7/2011 Roberts et al.       |  |  |
| 7,513,311 B2          | 4/2009 Gramstad et al.        | 7,987,906 B1 | 8/2011 Troy                 |  |  |
| 7,527,103 B2          | 5/2009 Huang et al.           | 7,992,763 B2 | 8/2011 Vecchio et al.       |  |  |
| 7,537,825 B1          | 5/2009 Wardle et al.          | 8,020,619 B1 | 9/2011 Robertson et al.     |  |  |
| 7,552,777 B2          | 6/2009 Murray et al.          | 8,020,620 B2 | 9/2011 Daniels et al.       |  |  |

(56)

## References Cited

## U.S. PATENT DOCUMENTS

|                 |         |                      |                 |         |                        |
|-----------------|---------|----------------------|-----------------|---------|------------------------|
| 8,025,104 B2    | 9/2011  | Cooke, Jr.           | 2003/0226668 A1 | 12/2003 | Zimmerman et al.       |
| 8,028,767 B2    | 10/2011 | Radford et al.       | 2004/0005483 A1 | 1/2004  | Lin                    |
| 8,033,331 B2    | 10/2011 | Themig               | 2004/0020832 A1 | 2/2004  | Richards et al.        |
| 8,039,422 B1    | 10/2011 | Al-Zahrani           | 2004/0031605 A1 | 2/2004  | Mickey                 |
| 8,056,628 B2    | 11/2011 | Whitsitt et al.      | 2004/0045723 A1 | 3/2004  | Slup et al.            |
| 8,056,638 B2    | 11/2011 | Clayton et al.       | 2004/0055758 A1 | 3/2004  | Brezinski et al.       |
| 8,109,340 B2    | 2/2012  | Doane et al.         | 2004/0058167 A1 | 3/2004  | Arbab et al.           |
| 8,127,856 B1    | 3/2012  | Nish et al.          | 2004/0069502 A1 | 4/2004  | Luke                   |
| 8,153,052 B2    | 4/2012  | Jackson et al.       | 2004/0089449 A1 | 5/2004  | Walton et al.          |
| 8,163,060 B2    | 4/2012  | Imanishi et al.      | 2004/0094297 A1 | 5/2004  | Malone et al.          |
| 8,211,247 B2    | 7/2012  | Marya et al.         | 2004/0154806 A1 | 8/2004  | Bode et al.            |
| 8,211,248 B2    | 7/2012  | Marya                | 2004/0159428 A1 | 8/2004  | Hammond et al.         |
| 8,220,554 B2    | 7/2012  | Jordan et al.        | 2004/0159446 A1 | 8/2004  | Haugen et al.          |
| 8,226,740 B2    | 7/2012  | Chaumonnot et al.    | 2004/0182583 A1 | 9/2004  | Doane et al.           |
| 8,230,731 B2    | 7/2012  | Dyer et al.          | 2004/0216868 A1 | 11/2004 | Owen, Sr.              |
| 8,231,947 B2    | 7/2012  | Vaidya et al.        | 2004/0231845 A1 | 11/2004 | Cooke, Jr.             |
| 8,263,178 B2    | 9/2012  | Boulos et al.        | 2004/0251025 A1 | 12/2004 | Giroux et al.          |
| 8,276,670 B2    | 10/2012 | Patel                | 2004/0256109 A1 | 12/2004 | Johnson                |
| 8,277,974 B2    | 10/2012 | Kumar et al.         | 2004/0256157 A1 | 12/2004 | Tessari et al.         |
| 8,297,364 B2    | 10/2012 | Agrawal et al.       | 2004/0261993 A1 | 12/2004 | Nguyen                 |
| 8,327,931 B2    | 12/2012 | Agrawal et al.       | 2004/0261994 A1 | 12/2004 | Nguyen et al.          |
| 8,403,037 B2    | 3/2013  | Agrawal et al.       | 2005/0034876 A1 | 2/2005  | Doane et al.           |
| 8,413,727 B2    | 4/2013  | Holmes               | 2005/0051329 A1 | 3/2005  | Blaisdell              |
| 8,425,651 B2 *  | 4/2013  | Xu .....             | 2005/0064247 A1 | 3/2005  | Sane                   |
|                 |         | B22F 1/025           | 2005/0069449 A1 | 3/2005  | Jackson et al.         |
|                 |         | 75/245               | 2005/0074612 A1 | 4/2005  | Eklund et al.          |
| 8,459,347 B2    | 6/2013  | Stout                | 2005/0102255 A1 | 5/2005  | Atkins et al.          |
| 8,486,329 B2    | 7/2013  | Shikai et al.        | 2005/0106316 A1 | 5/2005  | Bultman                |
| 8,490,674 B2    | 7/2013  | Stevens et al.       | 2005/0126334 A1 | 6/2005  | Rigney et al.          |
| 8,490,689 B1    | 7/2013  | McClinton et al.     | 2005/0161212 A1 | 7/2005  | Mirchandani            |
| 8,535,604 B1    | 9/2013  | Baker et al.         | 2005/0161224 A1 | 7/2005  | Leismer et al.         |
| 8,573,295 B2    | 11/2013 | Johnson et al.       | 2005/0165149 A1 | 7/2005  | Starr et al.           |
| 8,631,876 B2    | 1/2014  | Xu et al.            | 2005/0194143 A1 | 9/2005  | Chanak et al.          |
| 8,663,401 B2    | 3/2014  | Marya et al.         | 2005/0199401 A1 | 9/2005  | Xu et al.              |
| 8,734,602 B2    | 5/2014  | Li et al.            | 2005/0205264 A1 | 9/2005  | Patel et al.           |
| 8,770,261 B2    | 7/2014  | Marya                | 2005/0205265 A1 | 9/2005  | Starr et al.           |
| 8,956,660 B2    | 2/2015  | Launag et al.        | 2005/0205266 A1 | 9/2005  | Todd et al.            |
| 8,978,734 B2    | 3/2015  | Stevens              | 2005/0235757 A1 | 9/2005  | Todd et al.            |
| 8,998,978 B2    | 4/2015  | Wang                 | 2005/0241824 A1 | 10/2005 | De Jonge et al.        |
| 9,057,242 B2    | 6/2015  | Mazyar et al.        | 2005/0241825 A1 | 11/2005 | Burris, II et al.      |
| 9,079,246 B2    | 7/2015  | Xu et al.            | 2005/0257936 A1 | 11/2005 | Burris, II et al.      |
| 9,080,098 B2    | 7/2015  | Xu et al.            | 2005/0268746 A1 | 11/2005 | Lehr                   |
| 9,089,408 B2    | 7/2015  | Xu                   | 2005/0269097 A1 | 12/2005 | Abkowitz et al.        |
| 9,260,935 B2    | 2/2016  | Murphree et al.      | 2005/0275143 A1 | 12/2005 | Towler                 |
| 10,016,810 B2 * | 7/2018  | Salinas .....        | 2005/0279501 A1 | 12/2005 | Toth                   |
| 2001/0040180 A1 | 11/2001 | Wittebrood et al.    | 2006/0012087 A1 | 1/2006  | Surjaatmadja et al.    |
| 2001/0045285 A1 | 11/2001 | Russell              | 2006/0013350 A1 | 1/2006  | Matsuda et al.         |
| 2001/0045288 A1 | 11/2001 | Allamon et al.       | 2006/0045787 A1 | 1/2006  | Akers                  |
| 2002/0000319 A1 | 1/2002  | Brunet               | 2006/0057479 A1 | 3/2006  | Jandeska et al.        |
| 2002/0007948 A1 | 1/2002  | Bayne et al.         | 2006/0081378 A1 | 4/2006  | Niimi et al.           |
| 2002/0014268 A1 | 2/2002  | Vann                 | 2006/0102871 A1 | 5/2006  | Wang                   |
| 2002/0020527 A1 | 2/2002  | Kilaas et al.        | 2006/0108114 A1 | 5/2006  | Johnson et al.         |
| 2002/0066572 A1 | 6/2002  | Muth                 | 2006/0108126 A1 | 5/2006  | Horn et al.            |
| 2002/0092654 A1 | 7/2002  | Coronado et al.      | 2006/0110615 A1 | 5/2006  | Karim et al.           |
| 2002/0096365 A1 | 7/2002  | Berscheidt et al.    | 2006/0116696 A1 | 6/2006  | Odermatt et al.        |
| 2002/0104616 A1 | 8/2002  | De et al.            | 2006/0124310 A1 | 6/2006  | Lopez De Cerdas et al. |
| 2002/0108756 A1 | 8/2002  | Harrall et al.       | 2006/0131011 A1 | 6/2006  | Lynde et al.           |
| 2002/0136904 A1 | 9/2002  | Glass et al.         | 2006/0131031 A1 | 6/2006  | McKeachnie et al.      |
| 2002/0139541 A1 | 10/2002 | Sheffield et al.     | 2006/0131081 A1 | 6/2006  | Mirchandani et al.     |
| 2002/0162661 A1 | 11/2002 | Krauss et al.        | 2006/0134312 A1 | 6/2006  | Rytlewski et al.       |
| 2003/0019639 A1 | 1/2003  | MacKay               | 2006/0144515 A1 | 7/2006  | Tada et al.            |
| 2003/0037925 A1 | 2/2003  | Walker et al.        | 2006/0150770 A1 | 7/2006  | Freim                  |
| 2003/0060374 A1 | 3/2003  | Cooke, Jr.           | 2006/0151178 A1 | 7/2006  | Howard et al.          |
| 2003/0075326 A1 | 4/2003  | Ebinger              | 2006/0153728 A1 | 7/2006  | Schoenung et al.       |
| 2003/0104147 A1 | 6/2003  | Bretschneider et al. | 2006/0162927 A1 | 7/2006  | Walker et al.          |
| 2003/0111728 A1 | 6/2003  | Thai et al.          | 2006/0169453 A1 | 8/2006  | Savery et al.          |
| 2003/0127013 A1 | 7/2003  | Zavitsanos et al.    | 2006/0186602 A1 | 8/2006  | Martin et al.          |
| 2003/0141060 A1 | 7/2003  | Hailey et al.        | 2006/0207763 A1 | 9/2006  | Hofman et al.          |
| 2003/0141061 A1 | 7/2003  | Hailey et al.        | 2006/0213670 A1 | 9/2006  | Bishop et al.          |
| 2003/0141079 A1 | 7/2003  | Doane et al.         | 2006/0231253 A1 | 10/2006 | Vilela et al.          |
| 2003/0150614 A1 | 8/2003  | Brown et al.         | 2006/0269437 A1 | 11/2006 | Pandey                 |
| 2003/0155114 A1 | 8/2003  | Pedersen et al.      | 2006/0283592 A1 | 12/2006 | Sierra et al.          |
| 2003/0155115 A1 | 8/2003  | Pedersen et al.      | 2007/0017674 A1 | 1/2007  | Blaisdell              |
| 2003/0159828 A1 | 8/2003  | Howard et al.        | 2007/0017675 A1 | 1/2007  | Hammami                |
| 2003/0164237 A1 | 9/2003  | Butterfield          | 2007/0029082 A1 | 2/2007  | Giroux et al.          |
| 2003/0183391 A1 | 10/2003 | Hriscu et al.        | 2007/0039161 A1 | 2/2007  | Garcia                 |
|                 |         |                      | 2007/0039741 A1 | 2/2007  | Hailey                 |
|                 |         |                      | 2007/0044958 A1 | 3/2007  | Rytlewski et al.       |

| (56)                  | References Cited |                        |                  |         |                          |  |  |
|-----------------------|------------------|------------------------|------------------|---------|--------------------------|--|--|
| U.S. PATENT DOCUMENTS |                  |                        |                  |         |                          |  |  |
| 2007/0044966 A1       | 3/2007           | Davies et al.          | 2009/0038858 A1  | 2/2009  | Griffo et al.            |  |  |
| 2007/0051521 A1       | 3/2007           | Fike et al.            | 2009/0044946 A1  | 2/2009  | Schasteen et al.         |  |  |
| 2007/0053785 A1       | 3/2007           | Hetz et al.            | 2009/0044949 A1  | 2/2009  | King et al.              |  |  |
| 2007/0054101 A1       | 3/2007           | Signalas et al.        | 2009/0050334 A1  | 2/2009  | Marya et al.             |  |  |
| 2007/0057415 A1       | 3/2007           | Katagiri et al.        | 2009/0056934 A1  | 3/2009  | Xu                       |  |  |
| 2007/0062644 A1       | 3/2007           | Nakamura et al.        | 2009/0065216 A1  | 3/2009  | Frazier                  |  |  |
| 2007/0074601 A1       | 4/2007           | Hong et al.            | 2009/0074603 A1  | 3/2009  | Chan et al.              |  |  |
| 2007/0074873 A1       | 4/2007           | McKeachnie et al.      | 2009/0084553 A1  | 4/2009  | Rytlewski et al.         |  |  |
| 2007/0102199 A1       | 5/2007           | Smith et al.           | 2009/0084556 A1  | 4/2009  | Richards et al.          |  |  |
| 2007/0107899 A1       | 5/2007           | Werner et al.          | 2009/0084600 A1  | 4/2009  | Severance                |  |  |
| 2007/0107908 A1       | 5/2007           | Vaidya et al.          | 2009/0090440 A1  | 4/2009  | Kellett et al.           |  |  |
| 2007/0108060 A1       | 5/2007           | Park                   | 2009/0107684 A1  | 4/2009  | Cooke, Jr.               |  |  |
| 2007/0119600 A1       | 5/2007           | Slup et al.            | 2009/0114381 A1  | 5/2009  | Stroobants               |  |  |
| 2007/0131912 A1       | 6/2007           | Simone et al.          | 2009/0114382 A1  | 5/2009  | Grove et al.             |  |  |
| 2007/0151009 A1       | 7/2007           | Conrad, III et al.     | 2009/0126436 A1  | 5/2009  | Fly et al.               |  |  |
| 2007/0151769 A1       | 7/2007           | Slutz et al.           | 2009/0139720 A1  | 6/2009  | Frazier                  |  |  |
| 2007/0169935 A1       | 7/2007           | Akbar et al.           | 2009/0145666 A1  | 6/2009  | Radford et al.           |  |  |
| 2007/0181224 A1       | 8/2007           | Marya et al.           | 2009/0151949 A1  | 6/2009  | Marya et al.             |  |  |
| 2007/0185655 A1       | 8/2007           | Le Bemadjiel           | 2009/0152009 A1  | 6/2009  | Slay et al.              |  |  |
| 2007/0187095 A1       | 8/2007           | Walker et al.          | 2009/0155616 A1  | 6/2009  | Thamida et al.           |  |  |
| 2007/0207182 A1       | 9/2007           | Weber et al.           | 2009/0159289 A1  | 6/2009  | Avant et al.             |  |  |
| 2007/0221373 A1       | 9/2007           | Murray                 | 2009/0178808 A1  | 7/2009  | Williamson et al.        |  |  |
| 2007/0221384 A1       | 9/2007           | Murray                 | 2009/0194273 A1  | 8/2009  | Surjaatmadja et al.      |  |  |
| 2007/0227745 A1       | 10/2007          | Roberts et al.         | 2009/0194745 A1* | 8/2009  | Tanaka ..... B23K 35/262 |  |  |
| 2007/0259994 A1       | 11/2007          | Tour et al.            |                  |         | 252/514                  |  |  |
| 2007/0261862 A1       | 11/2007          | Murray                 | 2009/0205841 A1  | 8/2009  | Kluge et al.             |  |  |
| 2007/0272411 A1       | 11/2007          | Lopez De Cerdas et al. | 2009/0211770 A1  | 8/2009  | Nutley et al.            |  |  |
| 2007/0272413 A1       | 11/2007          | Rytlewski et al.       | 2009/0226340 A1  | 9/2009  | Marya                    |  |  |
| 2007/0277979 A1       | 12/2007          | Todd et al.            | 2009/0226704 A1  | 9/2009  | Kauppinen et al.         |  |  |
| 2007/0284109 A1       | 12/2007          | East et al.            | 2009/0242202 A1  | 10/2009 | Rispler et al.           |  |  |
| 2007/0284112 A1       | 12/2007          | Magne et al.           | 2009/0242208 A1  | 10/2009 | Bolding                  |  |  |
| 2007/0299510 A1       | 12/2007          | Venkatraman et al.     | 2009/0242214 A1  | 10/2009 | Foster et al.            |  |  |
| 2008/0011473 A1       | 1/2008           | Wood et al.            | 2009/0255667 A1  | 10/2009 | Clem et al.              |  |  |
| 2008/0020923 A1       | 1/2008           | Debe et al.            | 2009/0255684 A1  | 10/2009 | Bolding                  |  |  |
| 2008/0047707 A1       | 2/2008           | Boney et al.           | 2009/0255686 A1  | 10/2009 | Richard                  |  |  |
| 2008/0060810 A9       | 3/2008           | Nguyen et al.          | 2009/0266548 A1  | 10/2009 | Olsen et al.             |  |  |
| 2008/0066923 A1       | 3/2008           | Xu                     | 2009/0260817 A1  | 11/2009 | Gambier et al.           |  |  |
| 2008/0066924 A1       | 3/2008           | Xu                     | 2009/0272544 A1  | 11/2009 | Giroux et al.            |  |  |
| 2008/0072705 A1       | 3/2008           | Chaumonnot et al.      | 2009/0283270 A1  | 11/2009 | Langeslag                |  |  |
| 2008/0078553 A1       | 4/2008           | George                 | 2009/0293672 A1  | 12/2009 | Mirchandani et al.       |  |  |
| 2008/0081866 A1       | 4/2008           | Gong et al.            | 2009/0301730 A1  | 12/2009 | Gweily                   |  |  |
| 2008/0093073 A1       | 4/2008           | Bustos et al.          | 2009/0305131 A1  | 12/2009 | Kumar et al.             |  |  |
| 2008/0099209 A1       | 5/2008           | Loretz et al.          | 2009/0308588 A1  | 12/2009 | Howell et al.            |  |  |
| 2008/0105438 A1       | 5/2008           | Jordan et al.          | 2009/0317556 A1  | 12/2009 | Macary                   |  |  |
| 2008/0115932 A1       | 5/2008           | Cooke                  | 2009/0317622 A1  | 12/2009 | Huang et al.             |  |  |
| 2008/0121390 A1       | 5/2008           | O'Malley et al.        | 2010/0003536 A1  | 1/2010  | Smith et al.             |  |  |
| 2008/0121436 A1       | 5/2008           | Slay et al.            | 2010/0012385 A1  | 1/2010  | Drivdahl et al.          |  |  |
| 2008/0127475 A1       | 6/2008           | Griffo                 | 2010/0015002 A1  | 1/2010  | Barrera et al.           |  |  |
| 2008/0135249 A1       | 6/2008           | Fripp et al.           | 2010/0015469 A1  | 1/2010  | Romanowski et al.        |  |  |
| 2008/0149325 A1       | 6/2008           | Crawford               | 2010/0025255 A1  | 2/2010  | Su et al.                |  |  |
| 2008/0149345 A1       | 6/2008           | Bicerano               | 2010/0032151 A1  | 2/2010  | Duphorne et al.          |  |  |
| 2008/0149351 A1       | 6/2008           | Marya et al.           | 2010/0034857 A1  | 2/2010  | Launag et al.            |  |  |
| 2008/0169105 A1       | 7/2008           | Williamson et al.      | 2010/0038076 A1  | 2/2010  | Spray et al.             |  |  |
| 2008/0169130 A1       | 7/2008           | Norman et al.          | 2010/0038595 A1  | 2/2010  | Imholt et al.            |  |  |
| 2008/0179060 A1       | 7/2008           | Surjaatmadja et al.    | 2010/0040180 A1  | 2/2010  | Kim et al.               |  |  |
| 2008/0179104 A1       | 7/2008           | Zhang et al.           | 2010/0044041 A1  | 2/2010  | Smith et al.             |  |  |
| 2008/0196801 A1       | 8/2008           | Zhao et al.            | 2010/0051278 A1  | 3/2010  | Mytopher et al.          |  |  |
| 2008/0202764 A1       | 8/2008           | Clayton et al.         | 2010/0055491 A1  | 3/2010  | Vecchio et al.           |  |  |
| 2008/0202814 A1       | 8/2008           | Lyons et al.           | 2010/0055492 A1  | 3/2010  | Barsoum et al.           |  |  |
| 2008/0210473 A1       | 9/2008           | Zhang et al.           | 2010/0089583 A1  | 4/2010  | Xu et al.                |  |  |
| 2008/0216383 A1       | 9/2008           | Pierick et al.         | 2010/0089587 A1  | 4/2010  | Stout                    |  |  |
| 2008/0223586 A1       | 9/2008           | Barnett                | 2010/0101803 A1  | 4/2010  | Clayton et al.           |  |  |
| 2008/0223587 A1       | 9/2008           | Cherewyk               | 2010/0116495 A1  | 5/2010  | Spray                    |  |  |
| 2008/0236829 A1       | 10/2008          | Lynde                  | 2010/0122817 A1  | 5/2010  | Surjaatmadja et al.      |  |  |
| 2008/0236842 A1       | 10/2008          | Bhavsar et al.         | 2010/0139930 A1  | 6/2010  | Patel et al.             |  |  |
| 2008/0248205 A1       | 10/2008          | Blanchet et al.        | 2010/0200230 A1  | 8/2010  | East, Jr. et al.         |  |  |
| 2008/0248413 A1       | 10/2008          | Ishii et al.           | 2010/0209288 A1  | 8/2010  | Marya                    |  |  |
| 2008/0264594 A1       | 10/2008          | Lohmueller et al.      | 2010/0236793 A1  | 9/2010  | Bjorgum                  |  |  |
| 2008/0277109 A1       | 11/2008          | Vaidya                 | 2010/0236794 A1  | 9/2010  | Duan et al.              |  |  |
| 2008/0277980 A1       | 11/2008          | Koda et al.            | 2010/0243254 A1  | 9/2010  | Murphy et al.            |  |  |
| 2008/0282924 A1       | 11/2008          | Saenger et al.         | 2010/0252273 A1  | 10/2010 | Duphorne                 |  |  |
| 2008/0296024 A1       | 12/2008          | Tianping et al.        | 2010/0252280 A1  | 10/2010 | Swor et al.              |  |  |
| 2008/0302538 A1       | 12/2008          | Hofman                 | 2010/0270031 A1  | 10/2010 | Patel                    |  |  |
| 2008/0314581 A1       | 12/2008          | Brown                  | 2010/0276136 A1  | 11/2010 | Evans et al.             |  |  |
| 2008/0314588 A1       | 12/2008          | Langlais et al.        | 2010/0276159 A1  | 11/2010 | Mailand et al.           |  |  |
|                       |                  |                        | 2010/0282338 A1  | 11/2010 | Gerrard et al.           |  |  |
|                       |                  |                        | 2010/0282469 A1  | 11/2010 | Richard et al.           |  |  |
|                       |                  |                        | 2010/0294510 A1  | 11/2010 | Holmes                   |  |  |
|                       |                  |                        | 2010/0297432 A1  | 11/2010 | Sherman et al.           |  |  |

| (56)                  | References Cited |                          |                          |               |                  |             |
|-----------------------|------------------|--------------------------|--------------------------|---------------|------------------|-------------|
| U.S. PATENT DOCUMENTS |                  |                          |                          |               |                  |             |
| 2010/0304182 A1       | 12/2010          | Facchini et al.          | 2013/0146144 A1          | 6/2013        | Joseph et al.    |             |
| 2010/0314105 A1       | 12/2010          | Rose                     | 2013/0146302 A1          | 6/2013        | Gaudette et al.  |             |
| 2010/0314126 A1       | 12/2010          | Kellner                  | 2013/0167502 A1*         | 7/2013        | Wilson .....     | B29C 70/025 |
| 2010/0319870 A1       | 12/2010          | Bewlay et al.            |                          |               |                  | 57/210      |
| 2010/0326650 A1       | 12/2010          | Tran et al.              | 2013/0168257 A1          | 7/2013        | Mazyar et al.    |             |
| 2011/0005773 A1       | 1/2011           | Dusterhoft et al.        | 2013/0186626 A1          | 7/2013        | Aitken et al.    |             |
| 2011/0036592 A1       | 2/2011           | Fay                      | 2013/0240200 A1          | 9/2013        | Frazier          |             |
| 2011/0048743 A1       | 3/2011           | Stafford et al.          | 2013/0240203 A1          | 9/2013        | Frazier          |             |
| 2011/0052805 A1       | 3/2011           | Bordere et al.           | 2013/0299185 A1          | 11/2013       | Xu et al.        |             |
| 2011/0056692 A1       | 3/2011           | Lopez De Cardenas et al. | 2013/0299192 A1          | 11/2013       | Xu et al.        |             |
| 2011/0056702 A1       | 3/2011           | Sharma et al.            | 2013/0300066 A1          | 11/2013       | Xu et al.        |             |
| 2011/0067872 A1       | 3/2011           | Agrawal                  | 2013/0319668 A1          | 12/2013       | Tschetter et al. |             |
| 2011/0067889 A1       | 3/2011           | Marya et al.             | 2013/0327540 A1          | 12/2013       | Hamid et al.     |             |
| 2011/0067890 A1       | 3/2011           | Themig                   | 2014/0014339 A1          | 1/2014        | O'Malley et al.  |             |
| 2011/0094406 A1       | 4/2011           | Marya et al.             | 2014/0027128 A1          | 1/2014        | Johnson et al.   |             |
| 2011/0100643 A1       | 5/2011           | Themig et al.            | 2014/0060834 A1          | 3/2014        | Quintero et al.  |             |
| 2011/0127044 A1       | 6/2011           | Radford et al.           | 2014/0116711 A1          | 5/2014        | Tang et al.      |             |
| 2011/0132143 A1       | 6/2011           | Xu et al.                | 2014/0186207 A1          | 7/2014        | Bae et al.       |             |
| 2011/0132612 A1       | 6/2011           | Agrawal et al.           | 2014/0190705 A1          | 7/2014        | Fripp et al.     |             |
| 2011/0132619 A1       | 6/2011           | Agrawal et al.           | 2014/0196899 A1          | 7/2014        | Jordan et al.    |             |
| 2011/0132620 A1       | 6/2011           | Agrawal et al.           | 2014/0262327 A1          | 9/2014        | Xu et al.        |             |
| 2011/0132621 A1       | 6/2011           | Agrawal et al.           | 2014/0360728 A1          | 12/2014       | Tashiro et al.   |             |
| 2011/0135530 A1       | 6/2011           | Xu et al.                | 2015/0060085 A1          | 3/2015        | Xu               |             |
| 2011/0135805 A1       | 6/2011           | Doucet et al.            | 2015/0065401 A1          | 3/2015        | Xu et al.        |             |
| 2011/0135953 A1       | 6/2011           | Xu et al.                | 2015/0240337 A1          | 8/2015        | Sherman et al.   |             |
| 2011/0136707 A1       | 6/2011           | Xu et al.                | 2015/0299838 A1          | 10/2015       | Doud et al.      |             |
| 2011/0139465 A1       | 6/2011           | Tibbles et al.           | 2016/0209391 A1          | 7/2016        | Zhang et al.     |             |
| 2011/0147014 A1       | 6/2011           | Chen et al.              | 2016/0258242 A1          | 9/2016        | Hayter et al.    |             |
| 2011/0186306 A1       | 8/2011           | Marya et al.             | 2017/0165745 A1          | 6/2017        | Salinas et al.   |             |
| 2011/0214881 A1       | 9/2011           | Newton                   | FOREIGN PATENT DOCUMENTS |               |                  |             |
| 2011/0247833 A1       | 10/2011          | Todd et al.              | CN                       | 1076968 A     | 10/1993          |             |
| 2011/0253387 A1       | 10/2011          | Ervin                    | CN                       | 1079234 A     | 12/1993          |             |
| 2011/0256356 A1       | 10/2011          | Tomantschger et al.      | CN                       | 1255879 A     | 6/2000           |             |
| 2011/0259610 A1       | 10/2011          | Shkurti et al.           | CN                       | 2658384 Y     | 11/2004          |             |
| 2011/0277987 A1       | 11/2011          | Frazier                  | CN                       | 1668545 A     | 9/2005           |             |
| 2011/0277989 A1       | 11/2011          | Frazier                  | CN                       | 101050417 A   | 10/2007          |             |
| 2011/0284232 A1       | 11/2011          | Huang                    | CN                       | 101351523 A   | 1/2009           |             |
| 2011/0284240 A1       | 11/2011          | Chen et al.              | CN                       | 101454074 A   | 6/2009           |             |
| 2011/0284243 A1       | 11/2011          | Frazier                  | CN                       | 101457321 A   | 6/2009           |             |
| 2011/0300403 A1       | 12/2011          | Vecchio et al.           | CN                       | 101605963     | 12/2009          |             |
| 2011/0314881 A1       | 12/2011          | Hatcher et al.           | CN                       | 101720378 A   | 6/2010           |             |
| 2012/0046732 A1       | 2/2012           | Sillekens et al.         | EP                       | 0033625 A1    | 8/1981           |             |
| 2012/0067426 A1       | 3/2012           | Soni et al.              | EP                       | 1174385 A2    | 1/2002           |             |
| 2012/0090839 A1       | 4/2012           | Rudic                    | EP                       | 1412175 A1    | 4/2004           |             |
| 2012/0103135 A1       | 5/2012           | Xu et al.                | EP                       | 1798301 A1    | 8/2006           |             |
| 2012/0107590 A1       | 5/2012           | Xu et al.                | EP                       | 1857570 A2    | 11/2007          |             |
| 2012/0118583 A1       | 5/2012           | Johnson et al.           | FR                       | 2782096 A1    | 2/2000           |             |
| 2012/0130470 A1       | 5/2012           | Agnew                    | GB                       | 912956 A      | 12/1962          |             |
| 2012/0145378 A1       | 6/2012           | Frazier et al.           | GB                       | 1046330 A     | 10/1966          |             |
| 2012/0145389 A1       | 6/2012           | Fitzpatrick, Jr.         | GB                       | 1280833 A     | 7/1972           |             |
| 2012/0168152 A1       | 7/2012           | Casciaro et al.          | GB                       | 1357065 A     | 6/1974           |             |
| 2012/0177905 A1       | 7/2012           | Seals et al.             | JP                       | 61067770 A    | 4/1986           |             |
| 2012/0205120 A1       | 8/2012           | Howell                   | JP                       | 754008 A      | 2/1995           |             |
| 2012/0205872 A1       | 8/2012           | Reinhardt et al.         | JP                       | 8232029 A     | 9/1996           |             |
| 2012/0211239 A1       | 8/2012           | Kritzler et al.          | JP                       | 2000185725 A1 | 7/2000           |             |
| 2012/0234546 A1       | 9/2012           | Xu et al.                | JP                       | 2002053902 A  | 2/2002           |             |
| 2012/0234547 A1       | 9/2012           | O'Malley et al.          | JP                       | 2004225084 A  | 8/2004           |             |
| 2012/0267101 A1       | 10/2012          | Cooke                    | JP                       | 2004225765 A  | 8/2004           |             |
| 2012/0269673 A1       | 10/2012          | Koo et al.               | JP                       | 2005076052 A  | 3/2005           |             |
| 2012/0292053 A1       | 11/2012          | Xu et al.                | JP                       | 2010502840 A  | 1/2010           |             |
| 2012/0318513 A1       | 12/2012          | Mazyar et al.            | KR                       | 950014350 B1  | 11/1995          |             |
| 2013/0004847 A1       | 1/2013           | Kumar et al.             | WO                       | 9909227 A1    | 2/1999           |             |
| 2013/0008671 A1       | 1/2013           | Booth et al.             | WO                       | 9947726 A1    | 9/1999           |             |
| 2013/0025409 A1       | 1/2013           | Xu                       | WO                       | 2004001087 A1 | 12/2003          |             |
| 2013/0029886 A1       | 1/2013           | Mazyar et al.            | WO                       | 2004073889 A1 | 9/2004           |             |
| 2013/0032357 A1       | 2/2013           | Mazyar et al.            | WO                       | 2005040068 A  | 5/2005           |             |
| 2013/0048304 A1       | 2/2013           | Agrawal et al.           | WO                       | 2007044635 A  | 4/2007           |             |
| 2013/0048305 A1       | 2/2013           | Xu et al.                | WO                       | 2007095376 A2 | 8/2007           |             |
| 2013/0052472 A1       | 2/2013           | Xu                       | WO                       | 2008034042 A3 | 3/2008           |             |
| 2013/0081814 A1       | 4/2013           | Gaudette et al.          | WO                       | 2008057045 A1 | 5/2008           |             |
| 2013/0084643 A1       | 4/2013           | Commarie et al.          | WO                       | 2008079485 A2 | 7/2008           |             |
| 2013/0105159 A1       | 5/2013           | Alvarez                  | WO                       | 2008079777 A2 | 7/2008           |             |
| 2013/0126190 A1       | 5/2013           | Mazyar et al.            | WO                       | 2009079745 A1 | 7/2009           |             |
| 2013/0133897 A1       | 5/2013           | Baihly et al.            | WO                       | 2010012184 A1 | 2/2010           |             |
| 2013/0144290 A1       | 6/2013           | Schiffl et al.           | WO                       | 2010083826    | 7/2010           |             |
|                       |                  |                          | WO                       | 2011071902 A2 | 6/2011           |             |
|                       |                  |                          | WO                       | 2011071907 A2 | 6/2011           |             |

(56)

## References Cited

## FOREIGN PATENT DOCUMENTS

|    |            |    |         |
|----|------------|----|---------|
| WO | 2011071910 | A2 | 6/2011  |
| WO | 2011130063 | A3 | 2/2012  |
| WO | 2012015567 | A2 | 2/2012  |
| WO | 2012149007 | A2 | 11/2012 |
| WO | 2012174101 | A2 | 12/2012 |
| WO | 2013053057 | A1 | 4/2013  |
| WO | 2013078031 | A1 | 5/2013  |
| WO | 2014121384 | A1 | 8/2014  |
| WO | 2016085798 |    | 6/2016  |

## OTHER PUBLICATIONS

- "Declaration of Karl T. Hartwig in Support of Petitioner Pursuant to 37 C.F.R. § 42.120", executed on Nov. 21, 2016 in support of U.S. Pat. No. 9,101,978, 51 pages.
- Callister, Jr., William D., Materials Science and Engineering an Introduction, Seventh Edition, 2006, pp. 111, 627, and G7.
- German, Randall M., Powder Metallurgy Science, Second Edition, 1994, 102 pages.
- Klar, Erhard, ASM Handbook: International Metals Handbook—Powder Metallurgy, vol. 7, 1997, pp. 14, 276, and 798.
- Petition for Inter Partes Review; Case No. IPR2017-00326; U.S. Pat. No. 9,101,978; Nov. 23, 2016; 46 pages.
- Petition for Inter Partes Review; Case No. IPR2017-00327; U.S. Pat. No. 8,573,295; Nov. 23, 2016; 53 pages.
- Schaffer, James P. et al., The Science and Design of Engineering Materials, Second Edition, 1999, pp. 122, 123, 098, and 699.
- Xie, Guoqiang et al., "TEM Observation of Interfaces between Particles in Al—Mg Alloy Powder Compacts Prepared by Pulse Electric Current Sintering", Materials Transactions, 2002, pp. 2177-2180, vol. 43—No. 9.
- "Baker Hughes Refines Expandable Tubular Technology with Abaqus and Insight", Simulia Realistic Simulation News, Jan./Feb. 2011, pp. 12-13.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Bakshi et al., "Carbon nanotube reinforced metal matrix composites—a review," International Materials Reviews; 2010, pp. 41-64, vol. 55, No. 1.
- Birbilis, et al., "Exploring Corrosion Protection of Mg Via Ionic Liquid Pretreatment", Surface & Coatings Technology; 201, pp. 4496-4504, (2007).
- Feng, et al., "Electroless Plating of Carbon Nanotubes with Silver" Journal of Materials Science, 39, (2004) pp. 3241-3243.
- Lee, et al., "Effects of Ni addition on hydrogen storage properties of Mg17Al12 alloy", Materials Chemistry and Physics, 2011, 126, pp. 319-324.
- Li, et al., "Investigation of aluminium-based nanocomposites with ultra-high strength", Materials Science and Engineering A, 527, pp. 305-316, (2009).
- Liu, et al.; "Electroless Nickel Plating on AZ91 Mg Alloy Substrate"; Surface & Coatings Technology; 200; pp. 5087-5093; (2006).
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Pardo, et al.; "Corrosion Behaviour of Magnesium/Aluminium Alloys in 3.5 wt% NaCl"; Corrosion Science; 50; pp. 823-834; (2008).
- Quik Drill Composite Frac Plug; Baker Hughes, Baker Oil Tools; Copyright 2002; 3 pages.
- Shi, et al.; "Influence of the Beta Phase on the Corrosion Performance of Anodised Coatings on Magnesium-Aluminium Alloys"; Corrosion Science; 47; pp. 2760-2777; (2005).
- Shimizu, et al., "Multi-walled carbon nanotube-reinforced magnesium alloy composites", Scripta Materialia, vol. 58, Issue 4, Feb. 2008, pp. 267-270.
- Shumbera, et al. "Improved Water Injector Performance in a Gulf of Mexico Deepwater Development Using an Openhole Frac Pack Completion and Downhole Filter System: Case History." SPE Annual Technical Conference and Exhibition, Oct. 5-8, 2003.
- Song, et al.; "Corrosion Mechanisms of Magnesium Alloys"; Advanced Engineering Materials; 1(1); pp. 11-33; (1999).
- Song, et al.; "Influence of Microstructure on the Corrosion of Diecast AZ91D"; Corrosion Science; 41; pp. 249-273; (1999).
- Song, et al.; "Understanding Magnesium Corrosion"; Advanced Engineering Materials; 5; No. 12; pp. 837-858; (2003).
- Sun, et al.; "Colloidal Processing of Carbon Nanotube/Alumina Composites" Chem. Mater. 2002, 14, pp. 5169-5172.
- Vickery, et al.; "New One-Trip Multi-Zone Frac Pack System with Positive Positioning." European Petroleum Conference, Oct. 29-31, 2002, Aberdeen, UK. [Abstract Only].
- Zeng, et al. "Progress and Challenge for Magnesium Alloys as Biomaterials," Advanced Engineering Materials, vol. 10, Issue 8, Aug. 2008, pp. B3-B14.
- Zhang, et al.; "High Strength Nanostructured Materials and Their Oil Field Applications"; Society of Petroleum Engineers; Conference Paper SPE 157092; SPE International Oilfield Nanotechnology Conference, 2012; 6 pages.
- Zhang, et al.; "Metal Coating on Suspended Carbon Nanotubes and its Implication to Metal-Tube Interaction", Chemical Physics Letters 331 (2000) 35-41.
- "Optisleeve Sliding Sleeve", [online]; [retrieved on Jun. 25, 2010]; retrieved from the Internet [weatherfordcorp/WFT033159.pdf](http://weatherford.com/weatherford/groups/.../weatherfordcorp/WFT033159.pdf).
- Baker Hughes, "Flow Control Systems," [online]; [retrieved on May 20, 2010]; retrieved from the Internet <http://www.bakerhughes.com/products-and-services/completions-and-productions/well-completions/packers-and-flow-control/flow-control-systems>.
- Bououdina, et al., "Comparative Study of Mechanical Alloying of (Mg+Al) and (Mg+Al+Ni) Mixtures for Hydrogen Storage", J. Alloys, Compds, 2002, 336, 222-231.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 6 pages.
- Coronado, "Development of an Internal Coiled Tubing Connector Utilizing Permanent Packer Technology"; Society of Petroleum Engineers, SPE Paper No. 46036; Apr. 15, 1998; 10 pages.
- Garfield, New One-Trip Sand-Control Completion System that Eliminates Formation Damage Resulting From conventional Perforating and Gravel-Pack Operations; SPE Annual Technical Conference and Exhibition, Oct. 9-12, 2005.
- Gray, et al., "Protective Coatings on Magnesium and Its Alloys—a Critical Review", Journal of Alloys and Compounds 336 (2002), pp. 88-113.
- Hsiao, et al., "Anodization of AZ91D Magnesium Alloy in Silicate-Containing Electrolytes"; Surface & Coatings Technology; 199; pp. 127-134; (2005).
- Hsiao, et al., "Characterization of Anodic Films Formed on AZ91D Magnesium Alloy"; Surface & Coatings Technology; 190; pp. 299-308; (2005).
- Huo et al.; "Corrosion of AZ91D Magnesium Alloy with a Chemical Conversion Coating and Electroless Nickel Layer"; Corrosion Science; 46; pp. 1467-1477; (2004).
- Kuzumaki, et al.; "Mechanical Characteristics and Preparation of Carbon Nanotube Fiber-Reinforced Ti Composite"; Advanced Engineering Materials, 2000, 2, No. 7.
- Liu, et al., "Calculated Phase Diagrams and the Corrosion of Die-Cast Mg—Al Alloys"; Corrosion Science, 2009, 51, 606-619.
- Lunder et al.; "The Role of Mg17Al12 Phase in the Corrosion of Mg Alloy AZ91"; Corrosion; 45(9); pp. 741-748; (1989).
- Majumdar, et al., "Laser Surface Engineering of a Magnesium Alloy with Al + Al2O3"; Surface and Coatings Technology 179 (2004) pp. 297-305.
- Murray, "Binary Alloy Phase Diagrams" Int. Met. Rev., 30(5) 1985 vol. 1, pp. 103-187.
- Nie, "Patents of Methods to Prepare Intermetallic Matrix Composites: A Review", Recent Patents on Materials Science 2008, vol. 1, pp. 232-240.

(56)

## References Cited

## OTHER PUBLICATIONS

- Saravanan et al., "Mechanically Alloyed Carbon Nanotubes (CNT) Reinforced Nanocrystalline AA 4032: Synthesis and Characterization," *Journal of Minerals & Materials Characterization & Engineering*, vol. 9, No. 11, pp. 1027-1035, 2010.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Song, "Recent Progress in Corrosion and Protection of Magnesium Alloys"; *Advanced Engineering Materials*; 7(7); pp. 563-586; (2005).
- Song, et al.; "A Possible Biodegradable Magnesium Implant Material," *Advanced Engineering Materials*, vol. 9, Issue 4, Apr. 2007, pp. 298-302.
- Song, et al.; "Corrosion Behaviour of AZ21, AZ501 and AZ91 in Sodium Chloride"; *Corrosion Science*; 40(10); pp. 1769-1791; (1998).
- Triolo et al., "Resolving the Completion Engineer's Dilemma: Permanent or Retrievable Packer?"; Society of Petroleum Engineers, SPE Paper No. 76711; May 20, 2002; 16 pages.
- Vernon Constien et al., "Development of Reactive Coatings to Protect Sand-Control Screens", SPE 112494, copyright 2008, Society of Petroleum Engineers, Presented at the 2008 SPE International Symposium and Exhibition on Formation Damage Control.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Wang, et al., "Contact-Damage-Resistant Ceramic/Single-Wall Carbon Nanotubes and Ceramic/Graphite Composites" *Nature Materials*, vol. 3, Aug. 2004, pp. 539-544.
- Watanabe, et al., "Superplastic Deformation Mechanism in Powder Metallurgy Magnesium Alloys and Composites", *Acta mater.* 49 (2001) pp. 2027-2037.
- Watarai, Trend of research and development for magnesium alloys—reducing the weight of structural materials in motor vehicles, (2006) Science and technology trends, Quaterly review No. 18, 84-97.
- Welch, et al., "Nonelastomeric Sliding Sleeve Maintains Long Term Integrity in HP/HT Application: Case Histories" [Abstract Only], SPE Eastern Regional Meeting, Oct. 23-25, 1996, Columbus, Ohio.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zhan, et al., "Single-wall carbon nanotubes as attractive toughening agents in alumina-based nanocomposites" *Nature Materials*, vol. 2., Jan. 2003, pp. 38-42.
- Zhang, et al.; "Formation of metal nanowires on suspended single-walled carbon nanotubes" *Applied Physics Letter*, vol. 77, No. 19 (2000), pp. 3015-3017.
- Zhang, et al.; "Study on the Environmentally Friendly Anodizing of AZ91D Magnesium Alloy"; *Surface and Coatings Technology*: 161; pp. 36-43; (2002).
- Zhu, et al., "The process of coating on ultrafine particles by surface hydrolysis reaction in a fluidized bed reactor", *Surface and Coatings Technology* 135 (2000) 14-17.
- Adams, et al.; "Thermal stabilities of aromatic acids as geothermal tracers", *Geothermics*, vol. 21, No. 3, 1992, pp. 323-339.
- Aviles et al., "Degradable Alternative to Risky Mill-Out Operations in Plug and Perf"; SPE-173695-MS; Society of Petroleum Engineers; SPE/ICOTA Coiled Tubing & Well Intervention Conference & Exhibition; Mar. 24-25, 2015; 10 Pages.
- Ayman, et al.; "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38 (2009), No. 2, pp. 1-5.
- Baker Hughes Incorporated. IN-Tallic Disintegrating Frac Balls. Houston: Baker Hughes Incorporated, 2011. Accessed Mar. 6, 2015.
- Baker Hughes, "Multistage", Oct. 31, 2011, BakerHughes.com; accessed Mar. 6, 2015.
- Bin et al., "Advances in Fluidization CVD Technology", East China University of Chemical Technology, China Academic Journal Electronic Publishing House, vol. 13, No. 4, Nov. 1992, pp. 360-365, English Abstract on p. 366.
- Chuan-Jun et al., "Study on Corrosion Kinetics of Mg—Ni alloys", *Journal of Kunming University of Science and Technology*, vol. 34, No. 5, pp. 10-13, Oct. 2009.
- International Search Report and Written Opinion, International Application No. PCT/US2016/041849, dated Oct. 26, 2016, Korean Intellectual Property Office; International Search Report 5 pages, Written Opinion 7 pages.
- Lin et al., "Processing and Microstructure of Nano-Mo/Al<sub>2</sub>O<sub>3</sub> Composites from MOCVD and Fluidized Bed", *Nanostructured Materials*, Nov. 1999, vol. 11, No. 8, pp. 1361-1377.
- M.S. Senthil Saravanan et al., "Mechanically Alloyed Carbon Nanotubes (CNT) Reinforced Nanocrystalline AA 4032: Synthesis and Characterization", *Journal of Minerals and Materials Characterization and Engineering*, vol. 9, No. 11 pp. 1027-1035 2010.
- Reid, Gary Carl, "Literature evaluation of induced groundwater tracers, field tracer techniques, and hydrodynamic dispersion values in porous media", *Theisiss in Geosciences (Masters)*, Texas Tech University, Aug. 1981, 109 pages.
- Rose, et al.; "The application of the polyaromatic sulfonates as tracers in geothermal reservoirs", *Geothermics* 30 (2001) pp. 617-640.
- Shigematsu, et al., "Surface Treatment of AZ91D Magnesium Alloy by Aluminum diffusion Coating", *Journal of Materials Science Letters* 19, 2000, pp. 473-475.
- Singh, et al., "Extended Homogeneity Range of Intermetallic Phases in Mechanically Alloyed Mg—Al Alloys", Elsevier Sciences Ltd., *Intermetallics* 11, 2003, pp. 373-376.
- Spencer et al., "Fluidized Bed Polymer Particle ALD Process for Producing HDPE/Alumina Nanocomposites", The 12th International Conference on Fluidization—New Horizons in Fluidization Engineering, vol. RP4 (2007).
- Stanley, et al.; "An Introduction to Ground-Water Tracers", Department of Hydrology and Water Resources, University of Arizona, Mar. 1985, pp. 1-219.
- Tsipas et al. "Effect of High Energy Ball Milling on Titanium-Hydroxyapatite Powders" *Powder Metallurgy*, Maney Publishing, London, GB, vol. 46, No. 1, Mar. 2003 (Mar. 2003), pp. 73-77.
- Zemel, "Tracers in the Oil Field", University of Texas at Austin, Center for Petroleum and Geosystems, Jan. 1995, Chapters 1, 2, 3, 7.
- "Sliding Sleeve", Omega Completion Technology Ltd, Sep. 29, 2009, retrieved on: [www.omega-completion.com](http://www.omega-completion.com).
- Ambat, et al., "Electroless Nickel-Plating on AZ91D Magnesium Alloy: Effect of Substrate Microstructure and Plating Parameters", *Surface and Coatings Technology*; 179; pp. 124-134; (2004).
- Baker Oil Tools, "Baker Oil Tools Introduces Revolutionary Sand Control Completion Technology," May 2, 2005.
- Baker Oil Tools, "Z-Seal Metal-to-Metal Expandable Sealing Device Uses Expanding Metal in Place of Elastomers," Nov. 6, 2006.
- Bastow, et al., "Clustering and formation of nano-precipitates in dilute aluminum and magnesium alloys", *Materials Science and Engineering*, 2003, C23, 757-762.
- Bercegeay, et al., "A One-Trip Gravel Packing System"; Society of Petroleum Engineers, Offshort Technology Conference, SPE Paper No. 4771; Feb. 7-8, 1974.
- Bybee, "One-Trip Completion System Eliminates Perforations," *Completions Today*, Sep. 2007, pp. 52-53.
- Chang, et al., "Electrodeposition of Aluminum on Magnesium Alloy in Aluminum Chloride (AlC13)-1-ethyl-3-methylimidazolium chloride (EMIC) Ionic Liquid and Its Corrosion Behavior"; *Electrochemistry Communications*; 9; pp. 1602-1606; (2007).
- Christoglou, et al., "Deposition of Aluminum on Magnesium by a CVD Process", *Surface and Coatings Technology* 184 (2004) 149-155.
- Constantine, "Selective Production of Horizontal Openhole Completions Using ECP and Sliding Sleeve Technology." SPE Rocky Mountain Regional Meeting, May 15-18, 1999, Gillette, Wyoming. [Abstract Only].

(56)

**References Cited****OTHER PUBLICATIONS**

- Curtin, et al., "CNT-reinforced ceramics and metals," Materials Today, 2004, vol. 7, pp. 44-49.
- Flahaut, et al., "Carbon Nanotube-Metal-Oxide Nanocomposites: Microstructure, Electrical Conductivity and Mechanical Properties" Acta amter. 48 (2000), pp. 3803-3812.
- Forsyth, et al.; "An Ionic Liquid Surface Treatment for Corrosion Protection of Magnesium Alloy AZ31"; Electrochem. Solid-State Lett. 2006 vol. 9, Issue 11, B52-B55/ 9(11); Abstract only; 1 page.
- Galanty, et al. "Consolidation of metal powders during the extrusion process," Journal of Materials Processing Technology (2002), pp. 491-496.
- Garfield, "Formation Damage Control Utilizing Composite-Bridge-Plug Technology for Monobore, Multizone Stimulation Operations," SPE 70004, 2001, Society of Petroleum Engineers Inc., This paper was prepared for presentation at the SPE Per.
- Garfield, et al., "Maximizing Inflow Performance in Soft Sand Completions Using New One-trip Sand Control Liner Completion Technology", SPE European Formation Damage Conference, May 25-27, 2005.
- Goh, et al., "Development of novel carbon nanotube reinforced magnesium nanocomposites using the powder metallurgy technique", Nanotechnology 17 (2006) 7-12.
- Han, et al., "Mechanical Properties of Nanostructured Materials", Rev. Adv. Mater. Sci. 9(2005) 1-16.
- Hermawan, et al., "Iron-manganese: new class of metallic degradable biomaterials prepared by powder metallurgy", Powder Metallurgy, vol. 51, No. 1, (2008), pp. 38-45.
- Hjortstam, et al. "Can we achieve ultra-low resistivity in carbon nanotube-based metal composites," Applied Physics A (2004), vol. 78, Issue 8, pp. 1175-1179.
- Hsiao, et al., "Baking Treatment Effect on Materials Characteristics and Electrochemical Behavior of anodic Film Formed on AZ91D Magnesium Alloy"; Corrosion Science; 49; pp. 781-793; (2007).
- Hsiao, et al., "Effect of Heat Treatment on Anodization and Electrochemical Behavior of AZ91D Magnesium Alloy"; J. Mater. Res.; 20(10); pp. 2763-2771;(2005).
- Lavernia, et al., "Cryomilled Nanostructured Materials: Processing and Properties", Materials Science and Engineering A, 493, (2008) pp. 207-214.
- Li, "Design of Abrasive Water Jet Perforation and Hydraulic Fracturing Tool," Oil Field Equipment, Mar. 2011.
- Maisano, "Cryomilling of Aluminum-Based and Magnesium-Based Metal Powders", Thesis, Virginia Tech, Jan. 13, 2006.
- Seyni, et al., "On the interest of using degradable fillers in co-ground composite materials", Powder Technology 190, (2009) pp. 176-184.
- Vahlas, et al., "Principles and Applications of CVD Powder Technology", Materials Science and Engineering R 53 (2006) pp. 1-72.

\* cited by examiner



FIG. 1



FIG. 2



FIG. 3

## 1

**METHODS OF MANUFACTURING  
DISSOLVABLE TOOLS VIA LIQUID-SOLID  
STATE MOLDING**

**BACKGROUND**

The disclosure is directed to methods of manufacturing dissolvable tools, and in particular to liquid-solid state molding methods of manufacturing dissolvable tools.

Oil and natural gas, or carbon dioxide sequestration wells often utilize wellbore components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> sequestration, etc.

To facilitate removal, such tools or components may be formed of a corrodible material so that they need not be physically removed by, for example, a mechanical operation, but may instead corrode or dissolve under downhole conditions.

Despite all the advances, the art is still receptive to alternative methods of manufacturing dissolvable tools, in particular methods having increased manufacturing capacity and reduced material cost.

**BRIEF DESCRIPTION**

A method of manufacturing a dissolvable article comprises: forming a liquid-solid mixture comprising secondary particles homogeneously dispersed in a molten metallic matrix material; disposing the liquid-solid mixture in a mold; agitating the liquid-solid mixture in the mold; and molding the liquid-solid mixture under agitation to form a dissolvable article, wherein the secondary particles and the metallic matrix material form a plurality of micro- or nano-sized galvanic cells in the dissolvable article.

Also disclosed is a dissolvable article comprising a metallic matrix comprising a plurality of grains formed from a metallic matrix material; the grains having a size of about 5 microns to about 300 microns; and secondary particles disposed on grain boundaries of the grains formed from the metallic matrix material; the secondary particles having a size of about 0.1 micron to about 2 microns; wherein the secondary particles and the metallic matrix material form a plurality of micro- or nano-sized galvanic cells in the dissolvable article.

**BRIEF DESCRIPTION OF THE DRAWINGS**

Referring now to the drawings wherein like elements are numbered alike in the several Figures:

FIG. 1 illustrates the microstructure of an article according to an embodiment of the disclosure;

FIG. 2 illustrates the microstructure of an article according to another embodiment of the disclosure; and

FIG. 3 illustrates the electrons' flowing directions during the dissolution of the article.

**DETAILED DESCRIPTION**

The inventors hereof have found that dissolvable tools can be made by liquid-solid state molding. The method increases the manufacture capacity as the size of the tools made from the method is almost unlimited. Moreover, the method has

## 2

reduced material cost. As a further advantageous feature, the dissolvable tools made from the method have adjustable and uniform dissolution rates.

The method comprises forming a liquid-solid mixture comprising secondary particles homogeneously dispersed in a molten metallic matrix material; disposing the liquid-solid mixture in a mold; agitating the liquid-solid mixture in the mold; and molding the liquid-solid mixture under agitation to form the dissolvable article.

The matrix material comprises one or more of the following: a magnesium-based alloy; an aluminum-based alloy; or a zinc-based alloy. As used herein, the term "metal-based alloy" means a metal alloy wherein the weight percentage of the specified metal in the alloy is greater than the weight percentage of any other component of the alloy, based on the total weight of the alloy.

Magnesium-based alloys suitable for use include alloys of magnesium with aluminum (Al), cadmium (Cd), calcium (Ca), cobalt (Co), copper (Cu), iron (Fe), manganese (Mn), nickel (Ni), silicon (Si), silver (Ag), strontium (Sr), thorium (Th), tungsten (W), zinc (Zn), zirconium (Zr), or a combination comprising at least one of these elements. Alloying or trace elements can be included in varying amounts to adjust the corrosion rate of the magnesium. Exemplary commercial magnesium-based alloys which include different combinations of the above alloying elements to achieve different degrees of corrosion resistance include but are not limited to, for example, those alloyed with aluminum, strontium, and manganese such as AJ62, AJ50x, AJ51x, and AJ52x alloys, and those alloyed with aluminum, zinc, and manganese such as AZ91A-E alloys. Other exemplary magnesium-based alloys include MgZrZn, MgAlZn, AlCuZnMn, and AlMg-ZnSiMn.

Aluminum-based alloys include all alloys that have aluminum as an alloy constituent. Exemplary aluminum alloys include Al—Cu alloy, Al—Mn alloy, Al—Si alloy, Al—Mg alloy, Al—Mg—Si alloy, Al—Zn alloy, Al—Li alloy, Al—Cu—Mg—X alloy, Al—Zn—Mg—Cu—X, where X represents alloying elements including Zn, Mn, Si, Cr, Fe, Ni, Ti, V, Cu, Pb, Bi, and Zr.

Zinc-based alloys include alloys of zinc with Al, Cu, Mg, Pb, Cd, Sn, Fe, Ni, Si, or a combination of the above elements. In a specific embodiment, the metallic matrix material is a magnesium alloy.

The metallic matrix material used to prepare the dissolvable article is in a particular form. The matrix particles have an initial average particle size from about 0.1  $\mu\text{m}$  to about 500  $\mu\text{m}$ , in an embodiment 0.5  $\mu\text{m}$  to about 250  $\mu\text{m}$ . The shape of the matrix particles may be regular or irregular. In an embodiment, the matrix particles may be, for example, spherical or oblong. Useful metallic matrix material has a corrosion rate of about 0.1 to about 200 mg/cm<sup>2</sup>/hour, specifically about 1 to about 150 mg/cm<sup>2</sup>/hour using aqueous 3 wt % KCl solution at 200° F. (93° C.).

The secondary particles, which have a lower reactivity relative to the metallic matrix material, acts as a cathode, whereas the metallic matrix, made of an alloy such as magnesium-based alloy which is more reactive than the secondary particles, is anodic relative to the secondary particles. A galvanic discharge cycle (e.g., corrosion) occurs between the relatively anodic and relatively cathodic materials in the presence of an electrolyte. By adjusting the compositions of the metallic matrix material and the secondary particles and the amount of the secondary particles relative to the metallic matrix, the corrosion rate of the dissolvable article is adjusted.

The secondary particles have a higher melting point as compared to the metallic matrix material so that the metallic matrix material can be selectively melted during the manufacturing process. In addition, the secondary particles and the metallic matrix material are selected such that they form micro- or nano-sized galvanic cells under the process conditions to make the dissolvable article. In particular, the secondary particles and the metallic matrix material are selected such that they do not form intermetallic compounds or a solid solution phase or only forms a solid solution phase with very small solubility under the process conditions so that all or a large portion (for example, greater than 90 wt. %, greater than about 95 wt. %, or greater than about 98 wt. %) of the secondary particles remain in their original composition and shape in the article. In an embodiment, less than about 10 wt. %, less than about 5 wt. %, or less than about 2 wt. % of secondary particles dissolve or form a solid solution phase or form an intermetallic compound with the metallic matrix material. Without wishing to be bound by theory, it is believed that if secondary particles react with the matrix material forming an intermetallic compound or solid solution and are fully consumed during the material processing, then the manufactured articles may not have galvanic cells thus are not dissolvable. Further without wishing to be bound by theory, it is believed that if less than 10 wt. % of secondary particles form a solid solution or intermetallic compound with the metallic matrix material during the process to prepare the dissolvable article, based on the total weight of the secondary particles, the articles prepared from such metallic matrix materials and secondary particles keep high chemical potential difference between the matrix and the secondary particles thus providing an article having a high dissolution rate.

Exemplary secondary particles include one or more of the following: a metal; an oxide of the metal; a nitride of the metal; or a cermet of the metal; wherein the metal is one or more of the following: W; Co; Cu; Ni; or Fe.

The amount of the secondary particles can vary depending on the specific materials used and desired corrosion rate. In an embodiment, the liquid-solid mixture comprises 0.01 to 10 wt. %, or 0.05 to 8 wt. %, or 0.1 to 6 wt. % of the secondary particles, based on the total weight of the liquid-solid mixture. In another embodiment, the weight ratio of the metallic matrix material relative to the secondary particles is about 99:1 to about 9:1 in the liquid-solid mixture.

One way to form the liquid-solid mixture is to mix the metallic matrix material in a solid form with the secondary particles to provide a blend; and heating the blend under agitation to selectively melt the metallic matrix material. Alternatively, the liquid solid mixture is made by heating the metallic matrix material in a solid form to provide a molten metallic matrix material; and introducing the secondary particles to the molten matrix material under agitation. Heating the blend and heating the metallic matrix material can be conducted at a temperature above the melting point of the metallic matrix material but below the melting point of the secondary particles. In an embodiment, the heating is to a temperature of about 600° C. to about 800° C. The heating can be conducted at atmospheric pressure in the presence or absence of an inert atmosphere. In another embodiment, less than about 10 wt. %, less than about 5 wt. %, less than about 2 wt. %, or less than about 1 wt % of the secondary particles dissolve under the process conditions.

To form a homogeneous liquid-solid mixture, an agitation force is applied to the metallic matrix material and the secondary particles. The agitation force can be generated by mechanical means, electromagnetic means, acoustic means,

or a combination comprising at least one of the foregoing. For example, the metallic matrix material and the secondary particles can be mechanically stirred in a crucible or a furnace. A magnetic field can also be applied to the metallic matrix material and the secondary particles. By randomly changing the field direction, the magnitude, and the frequency of the field, an agitation force is generated. Alternatively or in addition to mechanical and electromagnetic forces, an acoustic generator such as a megasonic energy source imparts wave energy to the metallic matrix material and the secondary particles and thus agitating them during the mixing.

The homogeneous liquid-solid mixture is then disposed in a mold. The method of disposing is not particularly limited. For example, the homogeneous liquid-solid mixture can be poured into the mold, pushed into the mold under a superatmospheric pressure, or drawn to the mold under a subatmospheric pressure.

The molding can be a pressure molding or a vacuum molding. In an embodiment the molding is conducted at a pressure of about 500 psi to about 30,000 psi or about 1000 psi to about 5000 psi. The pressure can be a superatmospheric pressure or a subatmospheric pressure. In an embodiment, the mold is not heated. In another embodiment, the mold is heated to a temperature of about 200° F. to about 800° F. or about 300° F. to about 600° F.

During the molding, an agitation force is applied to the mixture by mechanical means, electromagnetic means, acoustic means, or a combination comprising at least one of the foregoing. Without wishing to be bound by theory, it is believed that without agitation, the secondary particles may separate out from the metallic matrix material. As a result, the secondary particles may not be uniformly distributed throughout the molded product; and the dissolvable article would not have a uniform dissolution rate.

The mold product is allowed to cool down to room temperature when the mold is still under pressure. In the instance where the molded product is subjected to a subsequent extrusion operation, the molded product can be cooled to a temperature above the room temperature. An agitation force is also applied to the molded product during the cooling process. The cooled article can be machined and used as is.

For applications requiring higher strength, the molded article is further extruded. During extrusion, the pores inside the molded product are fully closed to provide a condensed article having high tensile strength, high shear strength, and high compression strength. In addition, the extruded product dissolves more uniformly. The extrusion temperature is about 600° F. to about 800° F.

The dissolvable article has a microstructure comprising a plurality of grains formed from the metallic matrix material. The grains have an average size of about 5 to about 300 microns. The size of the secondary particles is about 0.1 micron to about 2 microns. The variation of the average particle size of the secondary particles in the final dissolvable article and the average particle size of the secondary particles used to make the dissolvable article is less than about 10%, less than about 5% or less than about 2% based on the initial average particle size of the secondary particles. In an embodiment, the secondary particles are disposed only on the grain boundaries. In another embodiment, the secondary particles are disposed both on the grain boundaries and inside the grains.

The dissolvable article thus has micron-sized or nano-sized galvanic cells where the metallic matrix is the anode and the secondary particles are cathode. The dissolvable

article has uniform dissolution rate. In an embodiment, the dissolvable article has a corrosion rate of about 1 to about 300 mg/cm<sup>2</sup>/hour, specifically about 10 to about 200 mg/cm<sup>2</sup>/hour using aqueous 3 wt % KCl solution at 200° F. (93° C.).

FIGS. 1 and 2 illustrate the microstructures of articles according to some embodiments of the disclosure. The dissolvable article has a plurality of grains 10 formed from a metallic matrix material. The grains form grain boundaries 30. In FIG. 1, the secondary particles 20 are only disposed on grain boundaries. In FIG. 2, the secondary particles 20 are disposed on the grain boundaries as well inside the grains.

FIG. 3 shows a grain 10 and secondary particles 20 disposed in the grain. Because the metallic matrix material is more reactive than the secondary particles, the matrix material loses electrons and forms a cation. The electrons move from the metallic matrix material to the secondary particles. The direction of the electron movement is shown as 60 in FIG. 3. The cations formed from the matrix material dissolves in the electrolyte shown as 50 in FIG. 3. The presence of multiple micron-sized or nano-sized galvanic cells ensures that the reaction is conducted in a controllable manner.

Articles formed from the method disclosed herein are not particularly limited. Exemplary dissolvable articles include downhole articles such as a ball, a ball seat, a fracture plug, a bridge plug, a wiper plug, shear out plugs, a debris barrier, an atmospheric chamber disc, a swabbing element protector, a sealbore protector, a screen protector, a beaded screen protector, a screen basepipe plugs, a drill in stim liner plugs, ICD plugs, a flapper valve, a gaslift valve, a transmatic CEM plug, float shoes, darts, diverter balls, shifting/setting balls, ball seats, sleeves, teleperf disks, direct connect disks, drill-in liner disks, fluid loss control flappers, shear pins or screws, cementing plugs, teleperf plugs, drill in sand control beaded screen plugs, HP beaded frac screen plugs, hold down dogs and springs, a seal bore protector, a stimcoat screen protector, or a liner port plug.

All ranges disclosed herein are inclusive of the endpoints, and the endpoints are independently combinable with each other. As used herein, “combination” is inclusive of blends, mixtures, alloys, reaction products, and the like. All references are incorporated herein by reference.

The use of the terms “a” and “an” and “the” and similar referents in the context of describing the invention (especially in the context of the following claims) are to be construed to cover both the singular and the plural, unless otherwise indicated herein or clearly contradicted by context. “Or” means “and/or.” Further, it should further be noted that the terms “first,” “second,” and the like herein do not denote any order, quantity (such that more than one, two, or more than two of an element can be present), or importance, but rather are used to distinguish one element from another. The modifier “about” used in connection with a quantity is inclusive of the stated value and has the meaning dictated by the context (e.g., it includes the degree of error associated with measurement of the particular quantity). Unless defined otherwise, technical and scientific terms used herein have the same meaning as is commonly understood by one of skill in the art to which this invention belongs. As used herein, the size or average size of the particles refers to the largest dimension of the particles and can be determined by high resolution electron or atomic force microscope technology.

All references cited herein are incorporated by reference in their entirety. While typical embodiments have been set forth for the purpose of illustration, the foregoing descrip-

tions should not be deemed to be a limitation on the scope herein. Accordingly, various modifications, adaptations, and alternatives can occur to one skilled in the art without departing from the spirit and scope herein.

What is claimed is:

1. A method of manufacturing a dissolvable article, the method comprising:

10 forming a liquid-solid mixture comprising secondary particles dispersed in a molten metallic matrix material; disposing the liquid-solid mixture in a mold; agitating the liquid-solid mixture in the mold; molding the liquid-solid mixture under agitation to form a molded dissolvable article, wherein molding the liquid-solid mixture comprises applying a superatmospheric pressure of about 500 psi to about 30,000 psi to the liquid-solid mixture under agitation; cooling the molded dissolvable article; and applying an agitating force to the molded dissolvable article during cooling thus forming the dissolvable article;

20 wherein the secondary particles have an original shape and an original composition before being dispersed in the molten metallic matrix material, and greater than about 90 wt. % of the secondary particles remain in the original shape and the original composition in the dissolvable article; and

25 the secondary particles and the metallic matrix material form a plurality of micro- or nano-sized galvanic cells in the dissolvable article.

30 2. The method of claim 1 wherein less than 10 wt. % of the secondary particles form a solid solution, an intermetallic compound, or a combination thereof with the metallic matrix material, based on the total weight of the secondary particles.

35 3. The method of claim 1, wherein forming the liquid-solid mixture comprises:

40 mixing the metallic matrix material in a solid form with the secondary particles to provide a blend; and heating the blend under agitation to selectively melt the metallic matrix material.

45 4. The method of claim 1, wherein forming the liquid-solid mixture comprises:

46 heating the metallic matrix material in a solid form to provide a molten metallic matrix material; and introducing the secondary particles to the molten matrix material under agitation.

50 5. The method of claim 4, wherein heating the metallic matrix material is to a temperature of about 600° C. to about 700° C.

55 6. The method of claim 1, wherein agitating the liquid-solid mixture comprises applying an agitation force to the mixture by mechanical means, electromagnetic means, acoustic means, or a combination comprising at least one of the foregoing.

7. The method of claim 1, further comprising extruding the article.

60 8. The method of claim 1, wherein the metallic matrix material comprises one or more of the following: a magnesium-based alloy; an aluminum-based alloy; or a zinc-based alloy.

65 9. The method of claim 1, wherein the secondary particles comprise one or more of the following: a metal; an oxide of the metal; a nitride of the metal; or a cermet of the metal; wherein the metal is one or more of the following: W; Co; Cu; Ni; or Fe.

**10.** The method of claim 1, wherein the liquid-solid mixture comprises about 1 wt % to about 10 wt % of secondary particles, based on the total weight of the liquid solid mixture.

**11.** The method of claim 1, wherein the dissolvable article has a microstructure comprising a plurality of grains formed from the metallic matrix material.

**12.** The method of claim 11, wherein the secondary particles are disposed on grain boundaries of the grains formed from the metallic matrix material.

**13.** The method of claim 12, wherein the secondary particles are further disposed inside the grains.

**14.** The method of claim 1, wherein less than about 10 wt % of the secondary particles form an intermetallic compound with the metallic matrix material, based on the total weight of the secondary particles.

**15.** The method of claim 14, wherein less than about 5 wt % of the secondary particles form an intermetallic compound with the metallic matrix material, based on the total weight of the secondary particles.

**16.** The method of claim 1, wherein the secondary particles comprise one or more of the following: a metal; an oxide of the metal; a nitride of the metal; or a cermet of the metal; and the metal is W, Co, or a combination thereof.

**17.** The method of claim 1, wherein greater than about 95 wt % of the secondary particles remain in the original form shape and the original composition in the dissolvable article.

**18.** The method of claim 1, wherein greater than about 98 wt % of the secondary particles remain in the original shape and the original composition in the dissolvable article.

**19.** The method of claim 1, wherein the secondary particles comprise W, Co, or a combination thereof.

**20.** A method of manufacturing a dissolvable article, the method comprising:

forming a liquid-solid mixture comprising 0.1 to 6 wt % of secondary particles homogeneously dispersed in a molten metallic matrix material based on the total weight of the liquid-solid mixture, the metallic matrix material comprising one or more of the following: a magnesium-based alloy; an aluminum-based alloy; or a zinc-based alloy, and the secondary particles comprising a metal; an oxide of the metal; a nitride of the metal; or a cermet of the metal; wherein the metal is one or more of the following: W; Co; Cu; Ni; or Fe; disposing the liquid-solid mixture in a mold; agitating the liquid-solid mixture in the mold; molding the liquid-solid mixture under agitation to form a dissolvable molded article, wherein molding the liquid-solid mixture comprises applying a superatmospheric pressure of about 1,000 psi to about 5,000 psi to the liquid solid mixture under agitation; cooling the molded dissolvable article; and applying an agitating force to the molded dissolvable article during cooling thus forming the dissolvable article;

wherein the secondary particles have an original shape and an original composition before being dispersed in the molten metallic matrix material, and greater than about 98 wt % of the secondary particles remain in the original shape and the original composition in the dissolvable article; and

the secondary particles and the metallic matrix material form a plurality of micro- or nano-sized galvanic cells in the dissolvable article.

**21.** The method of claim 20, wherein the secondary particles comprise W, Co, or a combination thereof.

\* \* \* \* \*